



US01231255B2

(12) **United States Patent**  
**Ransom et al.**

(10) **Patent No.:** **US 12,312,555 B2**  
(45) **Date of Patent:** **May 27, 2025**

(54) **LUBRICATING COMPOSITION FOR DURABILITY AND ENHANCED FUEL ECONOMY**

(71) Applicant: **Afton Chemical Corporation**, Richmond, VA (US)

(72) Inventors: **Paul Ransom**, Huddersfield (GB); **Ian Bell**, Abingdon (GB); **Samuel Bruce Field**, Windsor (GB)

(73) Assignee: **Afton Chemical Corporation**, Richmond, VA (US)

(\*) Notice: Subject to any disclaimer, the term of this patent is extended or adjusted under 35 U.S.C. 154(b) by 0 days.

(21) Appl. No.: **18/629,441**

(22) Filed: **Apr. 8, 2024**

(65) **Prior Publication Data**

US 2024/0352376 A1 Oct. 24, 2024

**Related U.S. Application Data**

(60) Provisional application No. 63/495,909, filed on Apr. 13, 2023.

(51) **Int. Cl.**

**C10M 135/10** (2006.01)  
**C10M 135/18** (2006.01)  
**C10M 137/10** (2006.01)  
**C10M 141/10** (2006.01)  
**C10M 145/14** (2006.01)  
**C10M 161/00** (2006.01)  
**C10M 169/04** (2006.01)  
**C10N 20/02** (2006.01)  
**C10N 20/04** (2006.01)  
**C10N 30/00** (2006.01)  
**C10N 30/02** (2006.01)  
**C10N 30/04** (2006.01)  
**C10N 40/25** (2006.01)

(52) **U.S. Cl.**

CPC ..... **C10M 169/044** (2013.01); **C10M 135/10** (2013.01); **C10M 135/18** (2013.01); **C10M 137/10** (2013.01); **C10M 141/10** (2013.01); **C10M 145/14** (2013.01); **C10M 161/00** (2013.01); **C10M 2203/003** (2013.01); **C10M 2209/084** (2013.01); **C10M 2219/046** (2013.01); **C10M 2219/068** (2013.01); **C10M 2223/045** (2013.01); **C10N 2020/02** (2013.01); **C10N 2020/04** (2013.01); **C10N 2030/02** (2013.01); **C10N 2030/04** (2013.01); **C10N 2030/43** (2020.05); **C10N 2030/44** (2020.05);

**C10N 2030/45** (2020.05); **C10N 2030/52** (2020.05); **C10N 2030/54** (2020.05); **C10N 2040/25** (2013.01)

(58) **Field of Classification Search**

CPC ..... C10M 169/044; C10M 135/10; C10M 135/18; C10M 137/10; C10M 141/10; C10M 145/14; C10M 161/00; C10M 2203/003; C10M 2209/084; C10M 2219/046; C10M 2219/068; C10M 2223/045; C10N 2020/02; C10N 2020/04; C10N 2030/02; C10N 2030/04; C10N 2030/43; C10N 2030/44; C10N 2030/45; C10N 2030/52; C10N 2030/54

USPC ..... 508/365  
See application file for complete search history.

(56) **References Cited**

**U.S. PATENT DOCUMENTS**

2012/0302477 A1\* 11/2012 Langston ..... C10M 145/14 526/325  
2017/0101598 A1\* 4/2017 Cant ..... C10M 135/10  
2022/0162516 A1 5/2022 Fujita  
2022/0403284 A1 12/2022 Jones et al.

**FOREIGN PATENT DOCUMENTS**

WO 2021158757 A1 8/2021

**OTHER PUBLICATIONS**

Extended European Search Report for European Patent Application 24168086.7, dated Aug. 23, 2024.

\* cited by examiner

*Primary Examiner* — Prem C Singh

*Assistant Examiner* — Francis C Campanell

(74) *Attorney, Agent, or Firm* — Honigman LLP

(57) **ABSTRACT**

The present disclosure relates to engine lubricating oil compositions and methods of lubricating a diesel internal combustion engine effective to achieve robust performance in both durability (i.e., piston cleanliness) and improved fuel economy. In one aspect, the engine lubricating oil compositions herein have a composition effective to achieve passing piston cleanliness pursuant to CEC L-117-20 (i.e., the VW TDi3 test) and to achieve a positive fuel economy increase as measured pursuant to JASO M 366, and preferably a fuel economy improvement as measured pursuant to JASO M 366 of at least about 0.5 percent. The engine lubricating oil compositions herein may have a viscosity grade of 0W-8, 0W-12, 0W16, and/or 0W-20.

**19 Claims, No Drawings**

## 1

**LUBRICATING COMPOSITION FOR  
DURABILITY AND ENHANCED FUEL  
ECONOMY**

**CROSS-REFERENCE TO RELATED  
APPLICATION**

This Application claims priority under 35 U.S.C. 119 (e) to U.S. Provisional Application Ser. No. 63/495,909 filed on Apr. 13, 2023, the disclosure of which is hereby incorporated by reference in its entirety.

**TECHNICAL FIELD**

The present disclosure relates to lubricating compositions and, in particular, lubricating compositions exhibiting improved piston cleanliness with improved fuel economy.

**BACKGROUND**

Automotive manufacturers continue to the push for improved efficiency, fluid longevity, and fuel economy, and as such, demands on engines, lubricants, and their components continue to increase. Today's engines are often smaller, lighter and more efficient with technologies designed to improve fuel economy, performance, and power. These requirements also mean engine oil performance must evolve to meet the higher demands of such modern engines and their corresponding performance criteria tied to their unique use and applications. With such exacting demands for engine oils, lubricant manufacturers often tailor lubricants and their additives to meet certain performance requirements for industry and/or manufacturer applications.

Typically, industry standards and/or automotive manufacturers require certain performance such that a lubricant designed for one use or application may not satisfy all the requirements for a different use or application. For example, there are often tradeoffs in engine oil performance between fuel economy and durability (i.e., piston cleanliness). Fuel economy can be evaluated, for example, through the JASO M 366 fuel economy test, and durability can be evaluated through the VW TDi3 piston cleanliness test of CEC L-117-20. Formulations that are good for fuel economy tend to be detrimental to piston cleanliness and vice-versa. Such opposing criteria presents a challenge for the lubricant manufacturer.

**SUMMARY**

The present disclosure relates to engine lubricating oil compositions including one or more base oils of lubricating viscosity, wherein the one or more base oils have a combined base oil viscosity at 100° C. of less than or equal to about 5.4 cSt; a detergent system providing a minimum total base number (TBN), measured pursuant to ASTM D4739, to the engine lubricating oil composition of at least about 4 mg KOH/g; and wherein the engine lubricating oil composition has one or more of (i) a NOACK volatility of about 13% or less measured pursuant to CEC L-40-93 and/or ASTM D5800; (ii) a total base number (TBN) of the engine lubricating oil composition of about 10 or less mg KOH/g measured pursuant to ASTM D2896; (iii) a calculated sulfated ash content (SASH) of about 0.8 weight percent or less measured pursuant to ASTM D874; (iv) a CCS viscosity at -35° C. of about 6200 mPas or less measured pursuant to ASTM D5292; or (v) combinations thereof. Such embodiments of the engine lubricating oil compositions herein meet

## 2

or exceed lubricant performance set forth in the CEC L-117-20 (VW TDi3) piston cleanliness test, and preferably exhibit a piston cleanliness rating of at least about 53 merits, at least about 54 merits, at least about 55 merits, at least about 56 merits, at least about 57 merits, at least about 58 merits, or at least about 59 merits. Such embodiments of the engine lubricating oil compositions herein also have a positive fuel economy increase as measured pursuant to JASO M 366, and preferably exhibit a fuel economy improvement as measured pursuant to JASO M 366 of at least about 0.5%, at least about 0.6%, at least about 0.7%, or at least about 0.8%.

In other approaches or embodiments, the engine lubricating oil composition of the previous paragraph may include optional features or embodiments in any combination. These optional features or embodiments may include one or more of: wherein the detergent system is substantially free of phenate detergent additives; and/or wherein the detergent system comprises, consists of, or consists essentially of sulfonate detergent additives, and preferably the detergent system is only sulfonate detergent additives; and/or wherein the detergent system provides calcium, magnesium, or combinations thereof to the engine lubricating oil composition, and preferably, the detergent system includes only a magnesium-containing detergent additive; and/or wherein the detergent system provides about 800 to about 1800 ppm of magnesium to the engine lubricating oil composition, about 1000 to about 1500 ppm of magnesium, or about 1200 to about 1400 ppm of magnesium; and/or wherein the detergent system includes one or more overbased detergent additives having a total base number (TBN) as measured pursuant to ASTM D2896 of at least about 250 mg KOH/g, preferably at least about 300 mg KOH/g, more preferably at least about 350 mg KOH/g, or most preferably at least about 400 mg KOH/g; and/or wherein the engine lubricating oil composition has a TBN of about 8 or less measured pursuant to ASTM D2896; and/or wherein the TBN of the detergent system is about 4 to about 10 mg KOH/g as measured pursuant to ASTM D4739; and/or further comprising an oil-soluble molybdenum containing additive, preferably a molybdenum dialkyl dithiocarbamate compound; and/or further comprising molybdenum but no more than about 800 ppm of molybdenum, no more than about 700 ppm molybdenum, no more than about 600 ppm of molybdenum, no more than about 500 ppm of molybdenum, no more than about 400 ppm of molybdenum, no more than about 300 ppm of molybdenum, no more than about 200 ppm of molybdenum, no more than about 100 ppm of molybdenum, or no more than about 50 ppm of molybdenum; and/or further comprising one or more polymeric viscosity index improver additives, preferably about 2 to about 10 weight percent of the one or more polymeric viscosity index improver additives; and/or wherein the engine lubricating oil composition has a viscosity index of 130 to 300; and/or wherein the one or more polymeric viscosity index improver additive is one or (i) an olefin copolymer, (ii) a dispersant or a non-dispersant poly(meth)acrylate copolymer viscosity modifier having a weight average molecular weight of about 500,000 or less, or (iii) combinations thereof; and/or wherein the dispersant or the non-dispersant poly(meth)acrylate copolymer has a weight average molecular weight of about 200,000 to about 500,000 with a polydispersity index of about 1.5 to about 2.5 and includes (meth)acrylate monomer units with a hydrocarbyl group in the monomer ester moiety of up to about 700, up to about 1000, up to about 2000, up to about 4000, up to about 8000, or up to about 10000, or combinations thereof; and/or wherein the

engine lubricating oil composition is substantially free of polymeric viscosity index improver additives; and/or wherein the one or more base oils of lubricating viscosity is selected from an API group II base oil, an API Group III base oil, an API Group IV base oil, or mixtures thereof; and/or wherein the one or more base oils of lubricating viscosity is a gas-to-liquid (GTL) derived base oil, preferably a GTL base oil having a viscosity at 100° C. of 4 to 8 cSt; and/or wherein the engine lubricating oil composition has a viscosity grade of 0W-X, wherein X is preferably 8, 12, 16, 20, or 30; and/or wherein the engine lubricating oil composition has a viscosity grade of 0W-16; and/or wherein the base oil viscosity is about 5.2 cSt or less, about 5.1 cSt or less, about 5.0 cSt or less, about 4.8 cSt or less, about 4.5 cSt or less, or about 4.2 cSt or less; and/or wherein the base oil viscosity is at least about 3 cSt, at least about 3.2 cSt, at least about 3.4 cSt, at least about 3.6 cSt, or at least about 3.8 cSt; and/or wherein the engine lubricating oil composition further includes a dispersant inhibitor package, and wherein the dispersant inhibitor package preferably includes one or more of dispersants, detergents, antiwear additives, antioxidants, friction modifiers, pour point dispersants, seal swell agents, or combinations thereof; and/or further comprising about 5 to about 20 weight percent of a dispersant inhibitor package; and/or wherein the engine lubricating oil composition is substantially free of boron, substantially free of calcium, or combinations thereof; and/or further including one or more metal dihydrocarbyl dithiophosphate compounds, preferably one or more zinc dihydrocarbyl dithiophosphate compounds; and/or wherein the one or more metal dihydrocarbyl dithiophosphate compounds provide up to about 1000 ppm phosphorus to the lubricating oil composition, up to about 900 ppm phosphorus, or up to about 800 ppm phosphorus to the lubricating oil composition; and/or wherein the one or more metal dihydrocarbyl dithiophosphate compounds provide up to about 1000 ppm zinc to the lubricating oil composition, up to about 900 ppm zinc, or up to about 850 ppm phosphorus to the lubricating oil composition; and/or further comprising one or more sulfur-containing additives, and wherein the one or more sulfur-containing additives provide up to about 2500 ppm sulfur to the lubricating oil composition, up to about 2200 ppm sulfur, or up to about 2100 ppm sulfur to the lubricating oil composition.

In yet other approaches or embodiments, a method of 45 improving the fuel economy and the piston cleanliness of a passenger car engine using a lubricating oil composition is described herein. The method includes lubricating an engine crankcase of a passenger car engine with a lubricating oil composition; wherein the lubricating oil composition is set forth in any embodiment of this Summary; and wherein the lubricating oil composition meets or exceeds lubricant performance set forth in the CEC L-117-20 (VW TDi3) piston cleanliness test and the lubricating oil composition has a positive fuel economy increase as measured pursuant to 50 JASO M 366. In some embodiments, the method results in a piston cleanliness rating pursuant to CEC L-117-20 (VW TDi3) of at least about 53 merits, at least about 54 merits, at least about 55 merits, at least about 56 merits, at least about 57 merits, at least about 58 merits, or at least about 59 merits. In other embodiments, the methods result in a fuel economy improvement as measured pursuant to JASO M 366 of at least about 0.5%, at least about 0.6%, at least about 0.7%, or at least about 0.8%. In further embodiments or approaches of the method, any embodiment of the engine oil lubricating composition as described in this Summary may be used in the methods herein.

In yet further embodiments or approaches, methods of lubricating a crankcase of a passenger car engine using a lubricating oil composition is described herein. The methods may include lubricating an engine crankcase of a passenger car engine with a lubricating oil composition; wherein the lubricating oil composition is set forth in any embodiment of this Summary; and wherein the passenger car engine lubricated with the lubricating oil composition meets or exceeds lubricant performance set forth in the CEC L-117-20 (VW TDi3) piston cleanliness test and has a positive fuel economy increase as measured pursuant to JASO M 366.

In yet additional approaches or embodiments, any of the methods herein may include optional features, steps, or embodiments in any combination. These optional features, 15 step, or embodiments may include one or more of the following: wherein the lubricating oil composition has a piston cleanliness rating pursuant to CEC L-117-20 (VW TDi3) of at least about 53 merits, at least about 54 merits, at least about 55 merits, at least about 56 merits, at least about 57 merits, at least about 58 merits, or at least about 59 merits; and/or wherein the lubricating oil composition has a fuel economy improvement as measured pursuant to JASO M 366 of at least about 0.5%, at least about 0.6%, at least about 0.7%, or at least about 0.8%.

In yet further approaches or embodiments, the use of any embodiment of the engine oil lubricating composition of this Summary is described for achieving a piston cleanliness rating pursuant to CEC L-117-20 (VW TDi3) of at least 20 about 53 merits, at least about 54 merits, at least about 55 merits, at least about 56 merits, at least about 57 merits, at least about 58 merits, or at least about 59 merits and/or for achieving a fuel economy improvement as measured pursuant to JASO M 366 of at least about 0.5%, at least about 0.6%, at least about 0.7%, or at least about 0.8%.

35

#### DETAILED DESCRIPTION

The present disclosure relates to engine lubricating oil compositions and methods of lubricating a diesel internal combustion engine effective to achieve robust performance in both durability (i.e., piston cleanliness) and improved fuel economy. In one aspect, the engine lubricating oil compositions herein have a composition effective to achieve passing piston cleanliness pursuant to CEC L-117-20 (i.e., the VW TDi3 test) and to achieve a positive fuel economy increase as measured pursuant to JASO M 366, and preferably a fuel economy improvement as measured pursuant to JASO M 366 of at least about 0.5 percent. The engine lubricating oil compositions herein may have a viscosity grade of 0W-8, 0W-12, 0W16, and/or 0W-20. The compositions herein may be used in diesel engines.

In one approach or embodiment, the robust engine lubricating oil compositions described herein have select compositions to achieve both diesel durability and improved fuel 55 economy. In one aspect, the lubricating oil compositions herein include one or more base oils of lubricating viscosity, and in particular, one or more base oils having a combined base oil viscosity of less than or equal to about 5.4 cSt at 100° C. In another aspect, the lubricating oil compositions 60 herein also include a detergent system providing a minimum total base number (TBN), measured pursuant to ASTM D4739, to the engine lubricating oil composition of at least about 4 mg KOH/g. In yet further aspects, the engine lubricating oil compositions herein may also have a configuration effective to achieve one or more of (i) a NOACK volatility of about 13% or less measured pursuant to CEC L-40-63 and/or ASTM D5800; (ii) a total base number 65

(TBN) of about 10 or less mg KOH/g measured pursuant to ASTM D2896; (iii) a calculated sulfated ash content (SASH) of about 0.8 weight percent or less measured pursuant to ASTM D874; (iv) a CCS viscosity at  $-35^{\circ}\text{C}$ . of about 6200 mPas or less measured pursuant to ASTM D5292; and/or (v) combinations thereof.

So configured, the engine lubricating oil compositions meet or exceed lubricant performance set forth in the CEC L-117-20 (VW TDi3) piston cleanliness test, and preferably exhibit a piston cleanliness rating of at least about 53 merits, at least about 54 merits, at least about 55 merits, at least about 56 merits, at least about 57 merits, at least about 58 merits, or at least about 59 merits. At the same time, the engine lubricating oil compositions also achieve a positive fuel economy increase as measured pursuant to JASO M 366, and preferably a positive fuel economy improvement as measured pursuant to JASO M 366 of at least about 0.5%, at least about 0.6%, at least about 0.7%, or at least about 0.8%.

As discussed more below, the engine lubricating oil compositions herein achieve such performance through selection of one or more of specific base oil blend(s), a detergent system, and/or one or more polymeric viscosity index improver additives that work particular well in one or more viscosity grades of 0W-8, 0W-12, 0W16, and/or 0W-20. In some exemplary approaches, the lubricating oil compositions herein have an additive package contributing about 1000 to about 1800 ppm of magnesium, about 10 to about 60 ppm of molybdenum, about 500 to about 900 ppm of phosphorus, about 1500 to about 1900 ppm of sulfur, and/or about 500 to about 900 ppm of zinc. In other exemplary approaches, the additive packages herein may also provide a lubricant TBN (ASTM 4739) of greater than about 5 mg KOH/g and, preferably, about 5.2 to about 6.0 mg KOH/g and a SASH of about 0.7 to about 0.8. Further details on the lubricant componentry and additive packages is provided below and shown in the Examples herein.

#### The Detergent System

The engine lubricating oil compositions herein include select detergent systems configured to function with the noted base oil blends to achieve lubricant durability via the VW TDi3 piston cleanliness test with little to no phenate and, preferably no phenate detergent additives. In some approaches, the piston cleanliness is achieved with the detergents herein when minimum lubricant TBN levels (as measured through ASTM D4739) are maintained by sulfonate additives, which may be a blend of neutral, low-based, or overbased sulfonate detergents and, preferably, overbased magnesium and/or calcium-based sulfonate detergents. In some embodiments, preferred lubricant TBN levels (as measured through ASTM D4739) are at least about 4 mg KOH/g, at least about 5 mg KOH/g, at least about 7 mg KOH/g or at least about 8 mg/KOH/g and lubricant TBN levels (as measured through ASTM D4739) may be about 15 mg KOH/g or less, about 12 mg KOH/g or less, about 10 mg KOH/g or less, or about 9 mg KOH/g or less. ASTM D4739 generally evaluates the impact of detergent additives on the lubricant TBN levels. In other approaches, lubricant TBN levels, as measured through ASTM D2896, may be about 15 or less and, in other approaches, about 10 mg KOH/g or less and, as measured through ASTM D2896 may be about 6 mg KOH/g or higher, about 7 mg KOH/g or higher, or about 8 mg KOH/g or higher. ASTM D2896 generally evaluates the impact of all sources of a fluid's base number including detergents, dispersant, antiwear, antioxidants, and the like additives in the fluid. In embodiments, the detergent systems herein generally include one or more alkali or alkaline metal

salts of sulfonates with minor amounts of, residual levels of, or no other detergent additives such as phenates, calixarates, salixarates, salicylates, carboxylic acids, sulfurized derivatives thereof, or combinations thereof so long as the TBN levels and metal contents are maintained within desired ranges found favorable when combined with the selected base stocks discussed more below.

Suitable detergents and their methods of preparation are described in greater detail in numerous patent publications, including U.S. Pat. No. 7,732,390 and references cited therein, which are incorporated herein by reference. The lubricant compositions herein may include about 0.1 to about 5 weight percent of individual and/or total detergent additives, and in other approaches, about 0.15 to about 3 weight percent, and in yet other approaches, about 0.15 to 2.6 weight percent of individual and/or total detergent additives so long as the detergent additives meet the sulfonate amounts and other relationships noted herein.

As noted above and in some approaches, the detergent system provides select amounts of sulfonate additives and TBN levels with certain amounts of detergent metals (such as magnesium and/or calcium and, preferably, magnesium only). For instance, the detergent systems herein may provide an amount of total detergent metals that is greater than about 1000 ppm total metal based on the total lubricating composition, and in other approaches, about 1000 ppm to about 5000 ppm total metals, about 1200 ppm to about 3500 ppm total metal, or about 1300 to about 2500 ppm total metal. In other approaches, the detergent metals are calcium, sodium, and/or magnesium, and preferably calcium and/or magnesium provided by sulfonates and, more preferably, only calcium, sodium, and/or magnesium sulfonates. Most preferably, the metals are calcium, magnesium, or combinations thereof. In some embodiments, the detergent metals are preferably only magnesium provided by overbased magnesium sulfonate detergents.

Generally, suitable detergents in the system may include linear or branched alkali or alkaline earth metal salts, such as calcium, sodium, or magnesium, of petroleum sulfonic acids and long chain mono- or di-alkylaryl sulfonic acids with the aryl group being benzyl, tolyl, and xylyl and/or various phenates or derivatives of phenates. Examples of suitable detergents include, subject the required amounts of sulfonate, metals, and/or TBN levels, include the overbased variations of the following detergents: calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

The detergent additives may be neutral, low-based, or overbased and, preferably, overbased detergents as needed to meet the minimum detergent TBN numbers as noted

above. As understood, overbased detergent additives are well-known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The term "overbased" relates to metal salts, such as metal salts of sulfonates, carboxylates, salicylates and/or phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the MR is one and in an overbased salt, MR, is greater than one. They are commonly referred to as overbased, hyperbased, or superbased salts and may be salts of organic sulfur acids, carboxylic acids, or phenols.

As used herein, the term "TBN" is used to denote the Total Base Number in mg KOH/g as measured, for the lubricants as provided by the detergent systems herein, by the method of ASTM D4739. The detergent may be neutral or overbased and, as noted above, are overbased detergents. For example, a neutral detergent may have a total base number (TBN) of up to about 200 mg KOH/gram. In another example, an overbased detergent of the lubricating oil compositions herein may have a total base number (TBN) of about 200 mg KOH/gram or greater, or about 250 mg KOH/gram or greater, or about 350 mg KOH/gram or greater, or about 375 mg KOH/gram or greater, or about 400 mg KOH/gram or greater. The overbased detergent may have a metal to substrate ratio of from 1.1:1 or less, or from 2:1 or less, or from 4:1 or less, or from 5:1 or less, or from 7:1 or less, or from 10:1 or less, or from 12:1 or less, or from 15:1 or less, or from 20:1 or less.

Examples of suitable overbased detergents (so long as the sulfonate, TBN, metal amounts, and other relationships noted herein are satisfied) include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

Optionally, when a low-based or neutral detergent is incorporated into the detergent system, it generally has a TBN of up to 175 mg KOH/g, up to 150 mg KOH/g, up to 100 mg KOH/g, or up to 50 mg KOH/g. The low-based/neutral detergent may include a calcium or magnesium-containing detergent. Examples of suitable low-based/neu-

tral detergent (so long as the sulfonate soap and other relationships noted herein are satisfied) include, but are not limited to, calcium sulfonates, calcium phenates, calcium salicylates, magnesium sulfonates, magnesium phenates, and/or magnesium salicylates.

In some embodiments, the detergent additives used in the lubricants herein include at least an overbased calcium sulfonate, an overbased sodium sulfonate, and/or an overbased magnesium sulfonate with each having a total base number of 150 to 400 and, in other approaches, about 200 to 10 about 350. In other embodiments, the detergents herein are overbased calcium sulfonate and/or overbased magnesium sulfonate, and most preferably, only overbased magnesium sulfonate. The above described TBN values reflect those of 15 finished detergent components that have been diluted in a base oil.

In other embodiments, the TBN of the detergents herein may reflect a neat or non-diluted version of the detergent component. For example, the fluids herein may include 20 overbased calcium or sodium sulfonate as a neat additive having a TBN of about 300 to about 450, and in other approaches, about 380 to about 420, and/or overbased magnesium sulfonate as a neat additive having a TBN of about 500 to about 700, and in other approaches, about 600 to 25 about 700.

More specifically, the detergent systems herein include overbased calcium sulfonate and/or overbased magnesium sulfonate to achieve the detergent TBN as measured by 30 ASTM D4739 of at least about 4 mg KOH/g, at least about 5 mg KOH/g, at least about 6 mg KOH/g and the detergent TBN may be about 15 mg KOH/g or less, about 12 mg KOH/g or less, or about 10 mg KOH/g or less. Preferably, the detergent systems herein also provide at least one of calcium, magnesium, or combination thereof and most preferably only magnesium in amounts ranging from about 1000 to about 3,500 ppm of magnesium, about 1100 ppm to about 3,000 ppm, about 1200 ppm to about 2,000 ppm of magnesium, 1300 ppm to about 1,500 ppm of magnesium.

The detergent systems herein have select levels of 40 sulfonate soap content, and in particular at least about 75 percent sulfonate soap, and in other approaches, at least about 80 percent sulfonate soap, at least about 85 sulfonate soap, at least about 90 percent sulfonate soap, at least about 95 sulfonate soap, at least about 98 percent sulfonate soap, 45 at least about 99 percent sulfonate soap, or about 100 percent sulfonate soap (or any ranges therebetween).

In others approach, the detergent systems herein have a select weight ratio of sulfonate soap to phenate soap of about 50 75:25 or greater, about 80:20 or greater, about 85:15 or greater, about 90:10 or greater, or even about 95:5 or greater (wherein greater in context of the ratio means more sulfonate soap relative to the phenate soap). Preferably, the detergent systems herein only include residual levels, if any, of phenate soap, salicylate soap, calixarate soap, or soaps 55 other than sulfonate.

Soap content generally refers to the amount of neutral organic acid salt and reflects a detergent's cleansing ability, or detergency, and dirt suspending ability. The soap content of a lubricant can be determined by ASTM D3712. Further 60 discussion on determining soap content can be found in FUELS AND LUBRICANTS HANDBOOK, TECHNOLOGY, PROPERTIES, PERFORMANCE, AND TESTING, George Totten, editor, ASTM International, 2003, relevant portions thereof incorporated herein by reference.

#### 65 Dispersants

The lubricating compositions herein also include one or more optional dispersants and, preferably, higher molecular

weight dispersants. Dispersants are often known as ashless-type dispersants because, prior to mixing in a lubricating composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of suitable N-substituted long chain alkenyl succinimides for the lubricants herein include polyisobutylene succinimide dispersants with the number average molecular weight of the polyisobutylene substituent being in the range about 1,600 to about 50,000, or to about 5,000, or to about 3,000, or to about 2,500, or to about 2,200 as measured by GPC. Succinimide dispersants and their preparation are disclosed, for instance in U.S. Pat. No. 7,897,696 or U.S. Pat. No. 4,234,435, which are incorporated herein by reference. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethyleneamine).

In approaches, preferred amines for the dispersants may be selected from polyamines and hydroxylamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like. In some approaches, a so-called heavy polyamine may be used, which is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule.

In some embodiments, polyisobutylene (PIB), when included, is a preferred reactant to form the dispersants and may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

In some approaches, a HR-PIB having a number average molecular weight ranging from about 1,600 to about 3,000 may be suitable, as determined by GPC. Such HR-PIB is commercially available, or can be synthesized by the polymerization of isobutene in the presence of a non-chlorinated catalyst such as boron trifluoride, as described in U.S. Pat. No. 4,152,499 and/or U.S. Pat. No. 5,739,355. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696. In one embodiment, the present disclosure further comprises at least one dispersant derived from polyisobutylene succinic anhydride ("PIBSA"). The PIBSA may have an average of between about 1.0 and about 2.0 succinic acid moieties per polymer.

In some approaches, the dispersants in the lubricants herein may optionally be post-treated by conventional methods by a reaction with any of a variety of agents. Suitable post treat agents include boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. (See, e.g., U.S. Pat. Nos. 7,645,726; 7,214,649; 8,048,831; and 5,241,003, which are all incorporated herein by reference in their entirities.)

The boron compound used as a post-treating reagent can be selected from boron oxide, boron halides, boron acids and esters of boron acids in an amount to provide from about 0.1 atomic proportion of boron for each mole of the nitrogen composition to about 20 atomic proportions of boron for each atomic proportion of nitrogen used. In some approaches, the dispersant post-treated with boron may contain from about 0.05 weight percent to about 2.0 weight percent, or in other approaches, about 0.05 weight percent to about 0.7 weight percent boron, based on the total weight of the borated dispersant. In other approaches, the dispersants herein are not post-treated with a boron compound and the fluids have less than about 10 ppm or boron, less than about 5 ppm of boron, or preferably no amounts of boron.

In other approaches, carboxylic acid may also be used as a post-treating reagent and can be saturated or unsaturated mono-, di-, or poly-carboxylic acid. Examples of carboxylic acids include, but are not limited to, maleic acid, fumaric acid, succinic acid, and naphthalic diacid (e.g., 1,8-naphthalic diacid). Anhydrides can also be used as a post-treating reagent and can be selected from the group consisting of mono-unsaturated anhydride (e.g., maleic anhydride), alkyl or alkylene-substituted cyclic anhydrides (e.g., succinic anhydride or glutamic anhydride), and aromatic carboxylic anhydrides (including naphthalic anhydride, e.g., 1,8-naphthalic anhydride).

In one embodiment, the process of post-treating the dispersant includes first forming the succinimide product, as described above, and then further reacting the succinimide product with the post treating agent, such as a boron compound, such as boric acid. In some cases, the dispersants herein may be post-treated with more than one post-treatment agents. For example, the dispersant may be post-treated with a boron compound, such as boric acid, and also an anhydride, such as maleic anhydride and/or 1,8-naphthalic anhydride.

In approaches, the dispersant may be used in the lubricating composition in amounts from about 0.1 weight percent to about 15 weight percent, or about 0.1 weight percent to about 10 weight percent, about 0.1 weight percent to 8 weight percent, or about 1 weight percent to about 10 weight percent, or about 1 weight percent to about 8 weight percent, or about 1 weight percent to about 6 weight percent, based upon the final weight of the lubricating oil composition. Dispersants may provide at least about 400 ppm nitrogen and up to about 1,500 ppm nitrogen.

#### Oil Soluble Molybdenum Compounds

In some approaches, the engine lubricating oil compositions herein may optionally include one or more oil soluble molybdenum-containing compounds. The oil-soluble molybdenum compound may be any of molybdenum dithiocarbamates, molybdenum dialkyl dithiophosphates, molybdenum sulfides, molybdenum disulfides, molybdenum dithiophosphinates, amine salts of molybdenum compounds, molybdenum xanthates, molybdenum thioxanthates, molybdenum sulfides, molybdenum carboxylates,

molybdenum alkoxides, a trinuclear organo-molybdenum compound, and/or mixtures thereof. The molybdenum-containing compounds may be sulfur-containing or sulfur-free compounds. The molybdenum disulfide may be in the form of a stable dispersion.

In one embodiment the oil-soluble molybdenum compound may be selected from the group of molybdenum dithiocarbamates, molybdenum dialkyldithiophosphates, sulfur-free organomolybdenum complexes of organic amides, and mixtures thereof. In one embodiment, the oil-soluble molybdenum compound may be a molybdenum dithiocarbamate. Exemplary sulfur-free organomolybdenum complexes of organic amides are disclosed in U.S. Pat. No. 5,137,647.

In one approach or embodiment, suitable molybdenum dithiocarbamates may be represented by the Formula:



where  $R^5$ ,  $R^6$ ,  $R^7$ , and  $R^8$  are each, independently, a hydrogen atom, a  $C_1$  to  $C_{20}$  alkyl group, a  $C_6$  to  $C_{20}$  cycloalkyl, aryl, alkylaryl, or aralkyl group, or a  $C_3$  to  $C_{20}$  hydrocarbyl group optionally containing an ester, ether, alcohol, or carboxyl group; and  $X_1$ ,  $X_2$ ,  $Y_1$ , and  $Y_2$  are each, independently, a sulfur or oxygen atom. Examples of suitable groups for each of  $R^5$ ,  $R^6$ ,  $R^7$ , and  $R^8$  include 2-ethylhexyl, nonylphenyl, methyl, ethyl, n-propyl, iso-propyl, n-butyl, t-butyl, n-hexyl, n-octyl, nonyl, decyl, dodecyl, tridecyl, lauryl, oleyl, linoleyl, cyclohexyl and phenylmethyl. In other approaches,  $R^5$ ,  $R^6$ ,  $R^7$ , and  $R^8$  may each have  $C_6$  to  $C_{18}$  alkyl groups.  $X_1$  and  $X_2$  may be the same, and  $Y_1$  and  $Y_2$  may be the same.  $X_1$  and  $X_2$  may both comprise sulfur atoms, and  $Y_1$  and  $Y_2$  may both comprise oxygen atoms. Further examples of molybdenum dithiocarbamates include  $C_6$ - $C_{18}$  dialkyl or diaryldithiocarbamates, or alkyl-aryldithiocarbamates such as dibutyl-, diethyl-di-(2-ethylhexyl)-, dilauryl-, dioleyl-, and dicyclohexyl-dithiocarbamate.

Suitable examples of molybdenum compounds which may be used include commercial materials sold under the trade names such as Molyvan® 822, Molyvan® A, Molyvan® 2000, Molyvan® 807 and Molyvan® 855 from R. T. Vanderbilt Co., Ltd., and Sakura-Lube™ S-165, S-200, S-300, S-310G, S-525, S-600, S-700, and S-710 available from Adeka Corporation, and mixtures thereof. Suitable molybdenum components are described in U.S. Pat. Nos. 5,650,381; RE 37,363 E1; RE 38,929 E1; and RE 40,595 E1, incorporated herein by reference in their entireties.

In one embodiment and if included in the formulations, the molybdenum compound may be present in the engine lubricating oil composition in an amount to provide up to about 800 ppm of molybdenum, or about 5 ppm to 800 ppm molybdenum. As a further example, the molybdenum compound may be present in an amount to provide from about 30 to about 700 ppm molybdenum or from about 50 to 650 ppm molybdenum or from about 100 to 625 ppm molybdenum. In other approaches, the formulations herein may be devoid of the molybdenum dialkyl dithiocarbamate, and in this context, the formulations may have about 0.05 weight percent or less of the molybdenum dialkyl dithiocarbamate, about 0.01 weight percent or less, or none.

## Poly(meth)acrylate Copolymer

In another approach or embodiment, the engine lubricating oil compositions herein may include select poly(meth)acrylate copolymers. In some approaches, the select poly(meth)acrylate copolymers are configured to achieve a select viscosity index of the lubricants herein, and in other approaches, the select poly(meth)-acrylate copolymers may also have certain molecular weights and/or certain pendant side groups or arms that may be a blend of one or more distinct molecular weight pendant arms, such as low molecular weight, intermediate molecular weight, and/or high molecular weight pendant hydrocarbyl groups in ester moieties of (meth)acrylate monomer units forming the copolymer. In embodiments, the lubricants herein may include up to about 20 weight percent of the poly(meth)acrylate copolymers, in other approaches, about 3 to about 18 weight percent, about 3 to about 16 weight percent, about 3 to about 10 weight percent, or about 3 to about 8 weight percent. Polymer treat rates are provided on a liquid (diluted in base oil) basis unless otherwise indicated.

In one exemplary approach, a poly(meth)acrylate copolymer may have the structure of Formula I below with  $z$  being an integer sufficient to achieve a weight average molecular weight of about 20,000 to about 1,500,00 (in other approaches, about 100,000 to about 500,000, or about 200,000 to about 450,000, or about 200,000 to about 300,000) and wherein R is hydrogen if the monomer unit is an acrylate and a methyl group if the monomer unit is a methacrylate and R' is a liner or branched hydrocarbyl group sized to achieve the arm molecular weights as described herein:



Lubricants including the poly(meth)acrylate copolymers herein may have a viscosity index (as determined by ASTM D2270) of about 130 to about 300, in other approaches, about 150 to about 250, or about 150 to about 200, or more preferably about 180 to about 200. The poly(meth)acrylate copolymers herein may have different (meth)acrylate monomer units randomly spaced throughout the polymer as described below.

Monomers or reactants suitable to form this copolymer for the unique motorcycle fluids herein include at least one, and optionally, a blend of at least two distinct (meth)acrylate monomers or reactants selected from: (1) (meth)acrylate monomers with a low to intermediate weight average molecular weight hydrocarbyl group(s) in the ester moiety of up to about 700, or preferably, about 100 to about 700 or about 400 to about 700 and, optionally, (2) (meth)acrylate monomers with a high weight average molecular weight hydrocarbyl groups in the ester moiety of the monomers of about 6,000 to about 10,000 or about 6,000 to about 8,000. As used herein, "(meth)acrylate" refers to both methacrylate and/or acrylate monomers or monomer units (or mixtures). As also used herein, molecular weight of the ester hydrocarbyl groups in the monomer includes the hydrocarbyl chain as well as the ester oxygen, but does not include the carbonyl group.

Typically, the formed or resultant poly(meth)acrylate copolymers have monomer amounts effective to achieve a number average molecular weight of the total copolymer of about 20,000 or more, and in some instances, about 250,000 or less or about 200,000 or less, such as about 140,000 to about 240,000 or about 140,000 to about 200,000. The poly(meth)acrylate copolymer may also have a polydispersity index (Mw/Mn) of about 2.8 or less, or about 2.6 or less and, in other approaches, ranging from about 1.8 to about 2.6. In yet other approaches, the copolymers herein may have two differently sized pendant arms and, in such context, have a molecular weight ratio between higher and lower molecular weight arms of about 10:1 to about 50:1, in other approaches, about 11:1 to about 30:1, and in yet other approaches, about 12:1 to about 25:1. In other instances, the copolymers herein have a molecular weight ratio between higher and lower molecular weight arms of about 1.5:1 to about 25:1, and in other approaches, about 1.5:1 to about 16:1.

In approaches or embodiments, the poly(meth)acrylate copolymers herein include a reaction product in the form of a linear, random copolymer of select amounts of the low to intermediate and/or (optional) high molecular weight pendant hydrocarbyl (meth)acrylate monomers. These monomers and monomer units are described more below and include both linear and/or branched hydrocarbyl groups in the respective ester chains and, in some embodiments, form comb-like copolymers with at least one and, optionally, at least the two distinct molecular weight pendant arms.

In embodiments or approaches, the low molecular weight hydrocarbyl (meth)acrylate units or monomers are derived from alkyl (meth)acrylates with a linear or branched hydrocarbyl group in the ester moiety, and preferably a linear or branched alkyl group in the ester moiety, with a total carbon chain length of the monomer ester moiety (including any branching) from 6 to 20 carbons, and preferably, 12 to 16 carbons. An exemplary low molecular weight hydrocarbyl (meth)acrylate monomer may be lauryl (meth)acrylate that may include a blend of (meth)acrylate monomers or monomer units having alkyl chain lengths ranging from C12 to C16 and, in particular, alkyl chains of 12, 14, and 16 carbons in the blend, of which C12 alkyl (meth)acrylates are the majority. In other embodiments or approaches, the low or intermediate molecular weight hydrocarbyl (meth)acrylate units are derived from hydrocarbyl (meth)acrylate monomers with a hydrocarbyl group or a total hydrocarbyl ester length (including any branching) with a weight average molecular weight of at least about 500 and up to about 700. These molecular weight chains can be derived from olefins or, optionally, macromonomers of polymeric alcohols esterified with (meth)acrylic acid. The macromonomers may be derived from alkenes or alkadienes including ethylene, propylene, butene, butadiene, isoprene, or combinations thereof and have a molecular weight of about 700 or less, such as about 500 to about 700.

In yet other embodiments or approaches, the optional high molecular weight hydrocarbyl (meth)acrylate units or monomer are derived from hydrocarbyl (meth)acrylates with a hydrocarbyl group or a total hydrocarbyl ester length (including any branching) with a weight average molecular weight of at least about 6,000 and up to about 10,000 or about 6,000 to about 8,000. These high molecular weight chains can be derived from macromonomers of polymeric alcohols esterified with (meth)acrylic acid. The macromonomers may be derived from alkenes or alkadienes including ethylene, propylene, butene, butadiene, isoprene, or combinations thereof and have a molecular weight of about 10,000

or less or about 8,000 or less, such as about 500 to about 10,000, or about 6,000 to about 8,000.

In optional embodiments, the poly(meth)acrylate copolymers herein may also include other optional monomers and monomer units including, for instance, hydroxyalkyl (meth)acrylate and/or various dispersant monomers and monomer units. The poly(meth) acrylate copolymers herein may also optionally be functionalized with one or more dispersant monomer or monomer units; however, it is preferred that the poly(meth)acrylate copolymers are non-dispersant polymers and, thus, free-of or devoid of dispersant moieties as noted herein.

In one optional approach, a dispersant monomer or monomer unit may be nitrogen-containing monomers or units thereof. Such monomers, if used, may impart dispersant functionality to the polymer. In some approaches, the nitrogen-containing monomers may be (meth)acrylic monomers such as methacrylates, methacrylamides, and the like. In some approaches, the linkage of the nitrogen-containing moiety to the acrylic moiety may be through a nitrogen atom or alternatively an oxygen atom, in which case the nitrogen of the monomer will be located elsewhere in the monomer. The nitrogen-containing monomer may also be other than a (meth)acrylic monomer, such as vinyl-substituted nitrogen heterocyclic monomers and vinyl substituted amines. Nitrogen-containing monomers include those, for instance, in U.S. Pat. No. 6,331,603. Other suitable dispersant monomers include, but are not limited to, dialkylaminoalkyl acrylates, dialkylaminoalkyl (meth)acrylates, dialkylamino-alkyl acrylamides, dialkylaminoalkyl methacrylamides, N-tertiary alkyl acrylamides, and N-tertiary alkyl methacrylamides, where the alkyl group or aminoalkyl groups may contain, independently, 1 to 8 carbon atoms. For instance, the dispersant monomer may be dimethylaminoethyl(meth)acrylate. The nitrogen-containing monomer may be, for instance, t-butyl acrylamide, dimethylaminopropyl (meth)acrylamide, dimethylaminoethyl methacrylamide, N-vinyl pyrrolidone, N-vinylimidazole, or N-vinyl caprolactam. It may also be a (meth)acrylamide based on any of the aromatic amines disclosed in WO2005/087821 including 4-phenylazoaniline, 4-aminodiphenylamine, 2-aminobenzimidazole, 3-nitroaniline, 4-(4-nitrophenylazo)aniline, N-(4-amino-5-methoxy-2-methyl-phenyl)-benzamide, N-(4-amino-2,5-dimethoxy-phenyl)-benzamide, N-(4-amino-2,5-diethoxy-phenyl)-benzamide, N-(4-amino-phenyl)-benzamide, 4-amino-2-hydroxy-benzoic acid

The (meth)acrylate copolymers of the present disclosure are typically synthesized to have a number average molecular weight of about 20,000 or more, in other approaches, about 250,000 or less or about 200,000 or less. Suitable ranges for the number average molecular weights include, about 140,000 to about 250,000, and in other approaches, about 150,000 to about 200,000. Such copolymers herein typically have a polydispersity index ranging from about 1 to about 4, and in other approaches, about 1.2 to about 3.5, and in yet other approaches, about 1.5 to about 3, and in yet other approaches, about 1.6 to about 2.5.

The (meth)acrylate copolymers may be prepared by any suitable conventional or controlled free-radical polymerization technique. Examples include conventional free radical polymerization (FRP), reversible addition-fragmentation chain transfer (RAFT), atom transfer radical polymerization (ATRP), and other controlled types of polymerization known in the art. Polymerization procedures are known to those in the art and include, for instance, the use of common polymerization initiators (such as Vazo<sup>TM</sup> 67 (2.2'-Azobis (2-methylbutyronitrile), chain transfer agents (such as

dodecyl mercaptane) if using conventional FRP, or RAFT agents (such as 4-cyano-4-[(dodecylsulfanylthiocarbonyl)sulfanyl] pentanoic acid and the like) if using RAFT polymerization. Other initiators, chain transfer agents, RAFT agents, ATRP catalyst and initiator systems can be used as known in the art depending on the selected polymerization method as needed for a particular application.

Base Oil or Base Oil Blend:

The base oil used in the lubricating compositions herein may be oils of lubricating viscosity and selected from any of the base oils in API Groups I to V as specified in the American Petroleum Institute (API) Base Oil Interchangeability Guidelines. Preferably, the one or more base oils have a combined base oil viscosity (BOV) of less than or equal to about 5.4 cSt at 100° C. In some approaches, the one or more base oils of lubricating viscosity is selected from an API group II base oil, an API Group III base oil, an API Group IV base oil, or mixtures thereof. In yet other approaches, the one or more base oils of lubricating viscosity is a gas-to-liquid (GTL) derived base oil, preferably a GTL base oil having a viscosity at 100° C. of about 4 to about 8 cSt. In some approaches or embodiments, the combined base oil viscosity (BOV) of the base oil blends herein at 100° C. may be about 5.4 cSt or less, about 5.2 cSt or less, about 5.1 cSt or less, about 5.0 cSt or less, about 4.8 cSt or less, about 4.5 cSt or less, or about 4.2 cSt or less. In other approaches, the combined base oil viscosity of the base oil blends herein is at least about 3 cSt, at least about 3.2 cSt, at least about 3.4 cSt, at least about 3.6 cSt, or at least about 3.8 cSt. The five base oil groups are generally set forth in Table 1 below:

TABLE 1

| Base oil Category | Sulfur (%)                                          | Saturates (%) | Viscosity Index |
|-------------------|-----------------------------------------------------|---------------|-----------------|
| Group I           | >0.03                                               | and/or        | <90 80 to 120   |
| Group II          | ≤0.03                                               | and           | ≥90 80 to 120   |
| Group III         | ≤0.03                                               | and           | ≥90 ≥120        |
| Group IV          | All polyalphaolefins (PAOs)                         |               |                 |
| Group V           | All others not included in Groups I, II, III, or IV |               |                 |

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry. Group II+ may comprise high viscosity index Group II.

The base oil blend used in the disclosed lubricating oil composition may be a mineral oil, animal oil, vegetable oil, synthetic oil, synthetic oil blends, or mixtures thereof. Suitable oils may be derived from hydrocracking, hydrogenation, hydrofinishing, unrefined, refined, and re-refined oils, and mixtures thereof.

Unrefined oils are those derived from a natural, mineral, or synthetic source without or with little further purification treatment. Refined oils are similar to the unrefined oils

except that they have been treated in one or more purification steps, which may result in the improvement of one or more properties. Examples of suitable purification techniques are solvent extraction, secondary distillation, acid or base extraction, filtration, percolation, and the like. Oils refined to the quality of an edible may or may not be useful. Edible oils may also be called white oils. In some embodiments, lubricating oil compositions are free of edible or white oils.

10 Re-refined oils are also known as reclaimed or reprocessed oils. These oils are obtained similarly to refined oils using the same or similar processes. Often these oils are additionally processed by techniques directed to removal of spent additives and oil breakdown products.

15 Mineral oils may include oils obtained by drilling or from plants and animals or any mixtures thereof. For example such oils may include, but are not limited to, castor oil, lard oil, olive oil, peanut oil, corn oil, soybean oil, and linseed oil, as well as mineral lubricating oils, such as liquid 20 petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

25 Useful synthetic lubricating oils may include hydrocarbon oils such as polymerized, oligomerized, or interpolymerized olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as  $\alpha$ -olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl 30 alkanes, alkylated diphenyl ethers and alkylated diphenyl sulfides and the derivatives, analogs and homologs thereof or mixtures thereof. Polyalphaolefins are typically hydrogenated materials.

35 Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerized Fischer-Tropsch 40 hydrocarbons or waxes. In one embodiment oils may be prepared by a Fischer-Tropsch gas-to-liquid synthetic procedure as well as other gas-to-liquid oils.

45 The major amount of base oil included in a lubricating composition may be selected from the group consisting of Group I, Group II, a Group III, a Group IV, a Group V, and a combination of two or more of the foregoing, and wherein the major amount of base oil is other than base oils that arise from provision of additive components or viscosity index improvers in the composition. In another embodiment, the 50 major amount of base oil included in a lubricating composition may be selected from the group consisting of Group II, a Group III, a Group IV, a Group V, and a combination of two or more of the foregoing, and wherein the major amount of base oil is other than base oils that arise from provision of additive components or viscosity index improvers in the composition.

55 The amount of the oil of lubricating viscosity present may be the balance remaining after subtracting from 100 wt % the sum of the amount of the performance additives inclusive of viscosity index improver(s) and/or pour point depressant(s) and/or other top treat additives. For example, the oil of lubricating viscosity that may be present in a finished fluid

may be a major amount, such as greater than about 50 wt %, greater than about 60 wt %, greater than about 70 wt %, greater than about 80 wt %, greater than about 85 wt %, or greater than about 90 wt %.

The base oil systems herein, in some approaches or embodiments, include one or more of a Group I to Group V base oils and may have a KV100 of about 2 to about 20 cSt, in other approaches, about 2 to about 10 cSt, about 2.5 to about 6 cSt, in yet other approaches, about 2.5 to about 3.5 cSt, and in other approaches about 2.5 to about 4.5 cSt.

As used herein, the terms "oil composition," "lubrication composition," "lubricating oil composition," "lubricating oil," "lubricant composition," "fully formulated lubricant composition," "lubricant," and "lubricating and cooling fluid" are considered synonymous, fully interchangeable terminology referring to the finished lubrication product comprising a major amount of a base oil component plus minor amounts of the detergents and the other optional components.

#### Engine Lubricating Oil Compositions

The fully formulated engine oil compositions herein including the selected base oil blend, the detergent systems, the optional oil-soluble molybdenum compounds, and the selected poly(meth)acrylate copolymers as described above have a configuration such that the engine lubricating oil compositions have one or more of the following: (i) a NOACK volatility of about 13 percent or less measured pursuant to CEC L-40-63 and/or ASTM D5800 (preferably, about 12 to about 10 percent); (ii) a total base number (TBN) of about 10 or less mg KOH/g measured pursuant to ASTM D2896 (preferably, about 7 to about 9 mg KOH/g per ASTM D2896) and/or a total base number (TBN) of at least about 4 mg KOH/g measured pursuant to ASTM D4739 (preferably, about 4 to about 7 mg KOH/g per ASTM D4739); (iii) a calculated sulfated ash content (SASH) of about 0.8 weight percent or less measured pursuant to ASTM D874 (preferably, about 0.5 weight percent to about 0.8 weight percent); (iv) a CCS viscosity at -35° C. of about 6200 mPas or less measured pursuant to ASTM D5292 (preferably about 3000 to about 5800 mPas); and/or (v) combinations thereof. As noted above, when the engine lubricating oil compositions have such configuration and meet such performance parameters, the engine lubricating oil composition meets or exceeds lubricant durability performance set forth in the CEC L-117-20 (VW TDi3) piston cleanliness test, and preferably a piston cleanliness rating of at least about 53 merits, at least about 54 merits, at least about 55 merits, at least about 56 merits, at least about 57 merits, at least about 58 merits, or at least about 59 merits and the engine lubricating oil composition also has a positive fuel economy increase as measured pursuant to JASO M 366, preferably a fuel economy improvement as measured pursuant JASO M 366 of at least about 0.5%, at least about 0.6%, at least about 0.7%, or at least about 0.8%.

#### Optional Additives:

The lubricating oil compositions herein may also include a number of optional additives combined with the detergent systems, sulfurized additives, and boronated detergents as needed to meet performance standards. Those optional additives are described in the following paragraphs.

**Other Dispersants:** The lubricating oil composition may optionally include one or more other dispersants or mixtures thereof. Dispersants are often known as ashless-type dispersants because, prior to mixing in a lubricating oil composition, they do not contain ash-forming metals and they do not normally contribute any ash when added to a lubricant. Ashless type dispersants are characterized by a polar group

attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, as measured by GPC. Succinimide dispersants and their preparation are disclosed, for instance in U.S. Pat. No. 7,897,696 or U.S. Pat. No. 4,234,435. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethylene amine).

Preferred amines are selected from polyamines and hydroxylamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like.

A suitable heavy polyamine is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule. The heavy polyamine comprises more than 28 wt. % (e.g. >32 wt. %) total nitrogen and an equivalent weight of primary amine groups of 120-160 grams per equivalent.

In some approaches, suitable polyamines are commonly known as PAM and contain a mixture of ethylene amines where TEPA and pentaethylene hexamine (PEHA) are the major part of the polyamine, usually less than about 80%.

Typically, PAM has 8.7-8.9 milliequivalents of primary amine per gram (an equivalent weight of 115 to 112 grams per equivalent of primary amine) and a total nitrogen content of about 33-34 wt. %. Heavier cuts of PAM oligomers with practically no TEPA and only very small amounts of PEHA but containing primarily oligomers with more than 6 nitrogen atoms and more extensive branching, may produce dispersants with improved dispersancy.

In an embodiment the present disclosure further comprises at least one polyisobutylene succinimide dispersant derived from polyisobutylene with a number average molecular weight in the range about 350 to about 50,000, or to about 5000, or to about 3000, as determined by GPC. The polyisobutylene succinimide may be used alone or in combination with other dispersants.

In some embodiments, polyisobutylene, when included, may have greater than 50 mol %, greater than 60 mol %, 55 greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable 60 for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight 65 ranging from about 900 to about 3000 may be suitable, as determined by GPC. Such HR-PIB is commercially available, or can be synthesized by the polymerization of

isobutene in the presence of a non-chlorinated catalyst such as boron trifluoride, as described in U.S. Pat. No. 4,152,499 to Boerzel, et al. and U.S. Pat. No. 5,739,355 to Gateau, et al. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696.

In one embodiment, the present disclosure further comprises at least one dispersant derived from polyisobutylene succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This method is described in column 5 and 6 in U.S. Pat. No. 5,334,321.

The percent conversion of the polyolefin is calculated from the % actives using the equation in column 5 and 6 in U.S. Pat. No. 5,334,321.

Unless stated otherwise, all percentages are in weight percent and all molecular weights are number average molecular weights determined by gel permeation chromatography (GPC) using commercially available polystyrene standards (with a number average molecular weight of 180 to about 18,000 as the calibration reference).

In one embodiment, the dispersant may be derived from a polyalphaolefin (PAO) succinic anhydride. In one embodiment, the dispersant may be derived from olefin maleic anhydride copolymer. As an example, the dispersant may be described as a poly-PIBSA. In an embodiment, the dispersant may be derived from an anhydride which is grafted to an ethylene-propylene copolymer.

A suitable class of nitrogen-containing dispersants may be derived from olefin copolymers (OCP), more specifically, ethylene-propylene dispersants which may be grafted with maleic anhydride. A more complete list of nitrogen-containing compounds that can be reacted with the functionalized OCP are described in U.S. Pat. Nos. 7,485,603; 7,786,057; 7,253,231; 6,107,257; and 5,075,383; and/or are commercially available.

One class of suitable dispersants may also be Mannich bases. Mannich bases are materials that are formed by the condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may also be high molecular weight esters or half ester amides. A suitable dispersant may also be post-treated by conventional methods by a reaction with any of a variety of agents. Among these are boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 are incorporated herein by reference in their entireties.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003, hereby incorporated by reference. Such treatments include, treatment with: Inorganic phosphorous acids or anhydrides (e.g., U.S. Pat. Nos. 3,403,102 and 4,648,980); Organic phosphorous compounds (e.g., U.S. Pat. No.

3,502,677); Phosphorous pentasulfides; Boron compounds as already noted above (e.g., U.S. Pat. Nos. 3,178,663 and 4,652,387); Carboxylic acid, polycarboxylic acids, anhydrides and/or acid halides (e.g., U.S. Pat. Nos. 3,708,522 and 4,948,386); Epoxides polyepoxides or thioepoxides (e.g., U.S. Pat. Nos. 3,859,318 and 5,026,495); Aldehyde or ketone (e.g., U.S. Pat. No. 3,458,530); Carbon disulfide (e.g., U.S. Pat. No. 3,256,185); Glycidol (e.g., U.S. Pat. No. 4,617,137); Urea, thiourea or guanidine (e.g., U.S. Pat. Nos. 3,312,619; 3,865,813; and British Patent GB 1,065,595); Organic sulfonic acid (e.g., U.S. Pat. No. 3,189,544 and British Patent GB 2,140,811); Alkenyl cyanide (e.g., U.S. Pat. Nos. 3,278,550 and 3,366,569); Diketene (e.g., U.S. Pat. No. 3,546,243); A diisocyanate (e.g., U.S. Pat. No. 3,573,205); Alkane sultone (e.g., U.S. Pat. No. 3,749,695); 1,3-Dicarbonyl Compound (e.g., U.S. Pat. No. 4,579,675); Sulfate of alkoxylated alcohol or phenol (e.g., U.S. Pat. No. 3,954,639); Cyclic lactone (e.g., U.S. Pat. Nos. 4,617,138; 4,645,515; 4,668,246; 4,963,275; and 4,971,711); Cyclic carbonate or thiocarbonate linear monocarbonate or polycarbonate, or chloroformate (e.g., U.S. Pat. Nos. 4,612,132; 4,647,390; 4,648,886; 4,670,170); Nitrogen-containing carboxylic acid (e.g., U.S. Pat. No. 4,971,598 and British Patent GB 2,140,811); Hydroxy-protected chlorodicarbonyloxy compound (e.g., U.S. Pat. No. 4,614,522); Lactam, thiolactam, thiolactone or dithiolactone (e.g., U.S. Pat. Nos. 4,614,603 and 4,666,460); Cyclic carbonate or thiocarbonate, linear monocarbonate or polycarbonate, or chloroformate (e.g., U.S. Pat. Nos. 4,612,132; 4,647,390; 4,646,860; and 4,670,170); Nitrogen-containing carboxylic acid (e.g., U.S. Pat. No. 4,971,598 and British Patent GB 2,440,811); Hydroxy-protected chlorodicarbonyloxy compound (e.g., U.S. Pat. No. 4,614,522); Lactam, thiolactam, thiolactone or dithiolactone (e.g., U.S. Pat. Nos. 4,614,603, and 4,666,460); Cyclic carbamate, cyclic thiocarbamate or cyclic dithiocarbamate (e.g., U.S. Pat. Nos. 4,663,062 and 4,666,459); Hydroxyaliphatic carboxylic acid (e.g., U.S. Pat. Nos. 4,482,464; 4,521,318; 4,713,189); Oxidizing agent (e.g., U.S. Pat. No. 4,379,064); Combination of phosphorus pentasulfide and a polyalkylene polyamine (e.g., U.S. Pat. No. 3,185,647); Combination of carboxylic acid or an aldehyde or ketone and sulfur or sulfur chloride (e.g., U.S. Pat. Nos. 3,390,086; 3,470,098); Combination of a hydrazine and carbon disulfide (e.g., U.S. Pat. No. 3,519,564); Combination of an aldehyde and a phenol (e.g., U.S. Pat. Nos. 3,649,229; 5,030,249; 5,039,307); Combination of an aldehyde and an 0-diester of dithiophosphoric acid (e.g., U.S. Pat. No. 3,865,740); Combination of a hydroxyaliphatic carboxylic acid and a boric acid (e.g., U.S. Pat. No. 4,554,086); Combination of a hydroxyaliphatic carboxylic acid, then formaldehyde and a phenol (e.g., U.S. Pat. No. 4,636,322); Combination of a hydroxyaliphatic carboxylic acid and then an aliphatic dicarboxylic acid (e.g., U.S. Pat. No. 4,663,064); Combination of formaldehyde and a phenol and then glycolic acid (e.g., U.S. Pat. No. 4,699,724); Combination of a hydroxyaliphatic carboxylic acid or oxalic acid and then a diisocyanate (e.g., U.S. Pat. No. 4,713,191); Combination of inorganic acid or anhydride of phosphorus or a partial or total sulfur analog thereof and a boron compound (e.g., U.S. Pat. No. 4,857,214); Combination of an organic diacid then an unsaturated fatty acid and then a nitrosoaromatic amine optionally followed by a boron compound and then a glycolating agent (e.g., U.S. Pat. No. 4,973,412); Combination of an aldehyde and a triazole (e.g., U.S. Pat. No. 4,963,278); Combination of an aldehyde and a triazole then a boron compound (e.g., U.S. Pat. No. 4,981,492); Combination of cyclic lactone and a boron compound (e.g., U.S.

Pat. Nos. 4,963,275 and 4,971,711). The above-mentioned patents are herein incorporated in their entireties.

The TBN of a suitable dispersant may be from about 10 to about 65 mg KOH/g dispersant, on an oil-free basis, which is comparable to about 5 to about 30 TBN if measured on a dispersant sample containing about 50% diluent oil. TBN is measured by the method of ASTM D2896.

In yet other embodiments, the optional dispersant additive may be a hydrocarbyl substituted succinamide or succinimide dispersant. In approaches, the hydrocarbyl substituted succinamide or succinimide dispersant may be derived from a hydrocarbyl substituted acylating agent reacted with a polyalkylene polyamine and wherein the hydrocarbyl substituent of the succinamide or the succinimide dispersant is a linear or branched hydrocarbyl group having a number average molecular weight of about 250 to about 5,000 as measured by GPC using polystyrene as a calibration reference.

In some approaches, the polyalkylene polyamine used to form the dispersant has the Formula



wherein each R and R', independently, is a divalent C1 to C6 alkylene linker, each R<sub>1</sub> and R<sub>2</sub>, independently, is hydrogen, a C1 to C6 alkyl group, or together with the nitrogen atom to which they are attached form a 5- or 6-membered ring optionally fused with one or more aromatic or non-aromatic rings, and n is an integer from 0 to 8. In other approaches, the polyalkylene polyamine is selected from the group consisting of a mixture of polyethylene polyamines having an average of 5 to 7 nitrogen atoms, triethylenetetramine, tetraethylenepentamine, and combinations thereof.

The dispersant, if present, can be used in an amount sufficient to provide up to about 20 wt %, based upon the final weight of the lubricating oil composition. Another amount of the dispersant that can be used may be about 0.1 wt % to about 15 wt %, or about 0.1 wt % to about 10 wt %, about 0.1 to 8 wt %, or about 1 wt % to about 10 wt %, or about 1 wt % to about 8 wt %, or about 1 wt % to about 6 wt %, based upon the final weight of the lubricating oil composition. In some embodiments, the lubricating oil composition utilizes a mixed dispersant system. A single type or a mixture of two or more types of dispersants in any desired ratio may be used.

**Antioxidants:** The lubricating oil compositions herein also may optionally contain one or more antioxidants. Antioxidant compounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phe-

nol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., Irganox<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon atoms. Another commercially available hindered phenol antioxidant may be an ester and may include Ethanol<sup>TM</sup> 4716 available from Albemarle Corporation.

Useful antioxidants may include diarylamines and high molecular weight phenols. In an embodiment, the lubricating oil composition may contain a mixture of a diarylamine and a high molecular weight phenol, such that each antioxidant may be present in an amount sufficient to provide up to about 5%, by weight, based upon the final weight of the lubricating oil composition. In an embodiment, the antioxidant may be a mixture of about 0.3 to about 1.5% diarylamine and about 0.4 to about 2.5% high molecular weight phenol, by weight, based upon the final weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. Fatty acids and/or ester may be mixed with olefins, such as  $\alpha$ -olefins.

In another alternative embodiment the antioxidant composition also contains a molybdenum-containing antioxidant in addition to the phenolic and/or aminic antioxidants discussed above. When a combination of these three antioxidants is used, preferably the ratio of phenolic to aminic to molybdenum-containing component treat rates is (0 to 3):(0 to 3):(0 to 3).

The one or more antioxidant(s) may be present in ranges about 0 wt % to about 20 wt %, or about 0.1 wt % to about 10 wt %, or about 1 wt % to about 5 wt %, of the lubricating oil composition.

**Antiwear Agents:** The lubricating oil compositions herein also may optionally contain one or more antiwear agents. Examples of suitable antiwear agents include, but are not limited to, a metal thiophosphate; a metal dialkyldithiophosphate; a phosphoric acid ester or salt thereof; a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl)disulfides; and mixtures thereof. A suitable antiwear

agent may be a molybdenum dithiocarbamate. The phosphorus containing antiwear agents are more fully described in European Patent 612 839. The metal in the dialkyl phosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include titanium compounds, tartrates, tartrimides, oil soluble amine salts of phosphorus compounds, sulfurized olefins; (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl) disulfides. The tartrate or tartramide may contain alkyl-ester groups, where the sum of carbon atoms on the alkyl groups may be at least 8. The antiwear agent may in one embodiment include a citrate.

The antiwear agent may be present in ranges including about 0 wt % to about 15 wt %, or about 0.01 wt % to about 10 wt %, or about 0.05 wt % to about 5 wt %, or about 0.1 wt % to about 3 wt % of the lubricating oil composition.

**Boron-Containing Compounds:** The lubricating oil compositions herein may optionally contain one or more boron-containing compounds. Examples of boron-containing compounds include borate esters, borated fatty amines, borated epoxides, borated detergents, and borated dispersants, such as borated succinimide dispersants, as disclosed in U.S. Pat. No. 5,883,057. The boron-containing compound, if present, can be used in an amount sufficient to provide up to about 8 wt %, about 0.01 wt % to about 7 wt %, about 0.05 wt % to about 5 wt %, or about 0.1 wt % to about 3 wt % of the lubricating oil composition.

**Additional Detergents:** The lubricating oil composition may optionally further comprise one or more neutral, low based, or overbased detergents, and mixtures thereof. Suitable detergent substrates include phenates, sulfur containing phenates, sulfonates, calixarates, salixarates, salicylates, carboxylic acids, phosphorus acids, mono- and/or di-thiophosphoric acids, alkyl phenols, sulfur coupled alkyl phenol compounds, or methylene bridged phenols. Suitable detergents and their methods of preparation are described in greater detail in numerous patent publications, including U.S. Pat. No. 7,732,390 and references cited therein.

The detergent substrate may be salted with an alkali or alkaline earth metal such as, but not limited to, calcium, magnesium, potassium, sodium, lithium, barium, or mixtures thereof. In some embodiments, the detergent is free of barium. In some embodiments, a detergent may contain traces of other metals such as magnesium or calcium in amounts such as 50 ppm or less, 40 ppm or less, 30 ppm or less, 20 ppm or less, or 10 ppm or less. A suitable detergent may include alkali or alkaline earth metal salts of petroleum sulfonic acids and long chain mono- or di-alkylarylsulfonic acids with the aryl group being benzyl, tolyl, and xylyl. Examples of suitable detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, mag-

nesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergent additives are well known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The terminology "overbased" relates to metal salts, such as metal salts of sulfonates, carboxylates, and phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or superbased salts and may be salts of organic sulfur acids, carboxylic acids, or phenols.

An overbased detergent of the lubricating oil composition may have a total base number (TBN) of about 200 mg KOH/g or greater, or as further examples, about 250 mg KOH/g or greater, or about 350 mg KOH/g or greater, or about 375 mg KOH/g or greater, or about 400 mg KOH/g or greater. The TBN being measured by the method of ASTM D2896.

Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

The overbased calcium phenate detergents have a total base number of at least about 150 mg KOH/g, at least about 225 mg KOH/g, at least about 225 mg KOH/g to about 400 mg KOH/g, at least about 225 mg KOH/g to about 350 mg KOH/g or about 230 mg KOH/g to about 350 mg KOH/g, all as measured by the method of ASTM D2896. When such detergent compositions are formed in an inert diluent, e.g. a process oil, usually a mineral oil, the total base number reflects the basicity of the overall composition including diluent, and any other materials (e.g., promoter, etc.) that may be contained in the detergent composition.

The overbased detergent may have a metal to substrate ratio of from 1.1:1, or from 2:1, or from 4:1, or from 5:1, or from 7:1, or from 10:1. In some embodiments, a detergent is effective at reducing or preventing rust in an engine or other automotive part such as a transmission or gear. The detergent may be present in a lubricating composition at about 0 wt % to about 10 wt %, or about 0.1 wt % to about 8 wt %, or about 1 wt % to about 4 wt %, or greater than about 4 wt % to about 8 wt %.

Extreme Pressure Agents: The lubricating oil compositions herein also may optionally contain one or more extreme pressure agents. Extreme Pressure (EP) agents that are soluble in the oil include sulfur- and chlorosulfur-containing EP agents, chlorinated hydrocarbon EP agents and phosphorus EP agents. Examples of such EP agents include chlorinated wax; organic sulfides and polysulfides such as dibenzyl disulfide, bis(chlorobenzyl) disulfide, dibutyl tetrasulfide, sulfurized methyl ester of oleic acid, sulfurized alkyl phenol, sulfurized dipentene, sulfurized terpene, and sulfurized Diels-Alder adducts; phosphorusulfurized hydrocarbons such as the reaction product of phosphorus sulfide with turpentine or methyl oleate; phosphorus esters such as the dihydrocarbyl and trihydrocarbyl phosphites, e.g., dibutyl phosphite, diheptyl phosphite, dicyclohexyl phosphite, pentylphenyl phosphite; dipentylphenyl phosphite, tridecyl phosphite, distearyl phosphite and polypropylene substituted phenyl phosphite; metal thiocarbamates such as zinc dioctyldithiocarbamate and barium heptylphenol diacid; amine salts of alkyl and dialkylphosphoric acids, including, for example, the amine salt of the reaction product of a dialkyldithiophosphoric acid with propylene oxide; and mixtures thereof.

Friction Modifiers: The lubricating oil compositions herein also may optionally contain one or more friction modifiers. Suitable friction modifiers may comprise metal containing and metal-free friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanol-amides, phosphonates, metal-containing compounds, glycerol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate

(GMO) which may contain mono-, di-, and tri-esters of oleic acid. Other suitable friction modifiers are described in U.S. Pat. No. 6,723,685, herein incorporated by reference in its entirety.

5 Aminic friction modifiers may include amines or polyamines. Such compounds can have hydrocarbyl groups that are linear, either saturated or unsaturated, or a mixture thereof and may contain from about 12 to about 25 carbon atoms. Further examples of suitable friction modifiers include alkoxylated amines and alkoxylated ether amines. Such compounds may have hydrocarbyl groups that are linear, either saturated, unsaturated, or a mixture thereof. They may contain from about 12 to about 25 carbon atoms. Examples include ethoxylated amines and ethoxylated ether amines.

10 The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference in its entirety.

15 A friction modifier may optionally be present in ranges such as about 0 wt % to about 10 wt %, or about 0.01 wt % to about 8 wt %, or about 0.1 wt % to about 4 wt %.

20 Other Molybdenum-containing components: The lubricating oil compositions herein also may optionally contain one or more molybdenum-containing compounds. An oil-soluble molybdenum compound may have the functional 25 performance of an antiwear agent, an antioxidant, a friction modifier, or mixtures thereof. An oil-soluble molybdenum compound may include molybdenum dithiocarbamates, molybdenum dialkyldithiophosphates, molybdenum dithiophosphinates, amine salts of molybdenum compounds, 30 molybdenum xanthates, molybdenum thioxanthates, molybdenum sulfides, molybdenum carboxylates, molybdenum alkoxides, a trinuclear organo-molybdenum compound, and/or mixtures thereof. The molybdenum sulfides include 35 molybdenum disulfide. The molybdenum disulfide may be 40 in the form of a stable dispersion. In one embodiment the oil-soluble molybdenum compound may be selected from the group consisting of molybdenum dithiocarbamates, molybdenum dialkyldithiophosphates, amine salts of molybdenum compounds, and mixtures thereof. In one embodiment the oil-soluble molybdenum compound may be 45 a molybdenum dithiocarbamate.

50 Suitable examples of molybdenum compounds which may be used include commercial materials sold under the trade names such as Molyvan® 822, Molyvan® A, Molyvan® 2000 and Molyvan® 855 from R. T. Vanderbilt Co., Ltd., and Adeka Sakura-Lube® S-165, S-200, S-300, S-310G, S-525, S-600, S-700, and S-710 available from Adeka Corporation, and mixtures thereof. Suitable molybdenum components are described in U.S. Pat. No. 5,650, 55 381; US RE 37,363 E1; US RE 38,929 E1; and US RE 40,595 E1, incorporated herein by reference in their entireties.

60 Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate,  $MoOCl_4$ ,  $MoO_2Br_2$ ,  $Mo_2O_3Cl_6$ , molybdenum trioxide or similar acidic molybdenum compounds. Alternatively, the 65 compositions can be provided with molybdenum by molybdenum/sulfur complexes of basic nitrogen compounds as described, for example, in U.S. Pat. Nos. 4,263,152; 4,285,

822; 4,283,295; 4,272,387; 4,265,773; 4,261,843; 4,259,195 and 4,259,194; and WO 94/06897, incorporated herein by reference in their entireties.

Another class of suitable organo-molybdenum compounds are trinuclear molybdenum compounds, such as those of the formula  $\text{Mo}_3\text{S}_k\text{L}_n\text{Q}_z$  and mixtures thereof, wherein S represents sulfur, L represents independently selected ligands having organo groups with a sufficient number of carbon atoms to render the compound soluble or dispersible in the oil, n is from 1 to 4, k varies from 4 through 7, Q is selected from the group of neutral electron donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. Additional suitable molybdenum compounds are described in U.S. Pat. No. 6,723,685, herein incorporated by reference in its entirety.

The oil-soluble molybdenum compound may be present in an amount sufficient to provide about 0.5 ppm to about 2000 ppm, about 1 ppm to about 700 ppm, about 1 ppm to about 550 ppm, about 5 ppm to about 300 ppm, or about 20 ppm to about 250 ppm of molybdenum.

Transition Metal-containing compounds: In another embodiment, the oil-soluble compound may be a transition metal containing compound or a metalloid. The transition metals may include, but are not limited to, titanium, vanadium, copper, zinc, zirconium, molybdenum, tantalum, tungsten, and the like. Suitable metalloids include, but are not limited to, boron, silicon, antimony, tellurium, and the like.

In an embodiment, an oil-soluble transition metal-containing compound may function as antiwear agents, friction modifiers, antioxidants, deposit control additives, or more than one of these functions. In an embodiment the oil-soluble transition metal-containing compound may be an oil-soluble titanium compound, such as a titanium (IV) alkoxide. Among the titanium containing compounds that may be used in, or which may be used for preparation of the oil-soluble materials of, the disclosed technology are various Ti (IV) compounds such as titanium (IV) oxide; titanium (IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1,3-hexanedioate or titanium citrate or titanium oleate; and titanium (IV) (triethanolaminato)isopropoxide. Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium

compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl- (or alkyl) succinic anhydride. The resulting titanate-succinate intermediate may be used directly or it may be reacted with any of a number of materials, such as (a) a polyamine-based succinimide/amide dispersant having free, condensable —NH functionality; (b) the components of a polyamine-based succinimide/amide dispersant, i.e., an alkenyl- (or alkyl) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams+diluent oil) at 150° C. for 1.5 hours, to produce a titanium-modified succinimide dispersant.

Another titanium containing compound may be a reaction product of titanium alkoxide and  $\text{C}_6$  to  $\text{C}_{25}$  carboxylic acid. The reaction product may be represented by the following formula:



wherein n is an integer selected from 2, 3 and 4, and R is a hydrocarbyl group containing from about 5 to about 24 carbon atoms, or by the formula:



wherein m+n=4 and n ranges from 1 to 3,  $\text{R}_4$  is an alkyl moiety with carbon atoms ranging from 1-8,  $\text{R}_1$  is selected from a hydrocarbyl group containing from about 6 to 25 carbon atoms, and  $\text{R}_2$  and  $\text{R}_3$  are the same or different and are selected from a hydrocarbyl group containing from about 1 to 6 carbon atoms, or the titanium compound may be represented by the formula:



wherein x ranges from 0 to 3, R<sub>1</sub> is selected from a hydrocarbyl group containing from about 6 to 25 carbon atoms, R<sub>2</sub>, and R<sub>3</sub> are the same or different and are selected from a hydrocarbyl group containing from about 1 to 6 carbon atoms, and R<sub>4</sub> is selected from a group consisting of either H, or C<sub>6</sub> to C<sub>25</sub> carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium by weight or 25 to about 1500 ppm titanium by weight or about 35 ppm to 500 ppm titanium by weight or about 50 ppm to about 300 ppm.

Other Viscosity Index Improvers: The lubricating oil compositions herein also may optionally contain one or more viscosity index improvers. Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, or mixtures thereof. Viscosity index improvers may include star polymers and suitable examples are described in US Publication No. 20120101017A1.

The lubricating oil compositions herein also may optionally contain one or more dispersant viscosity index improvers in addition to a viscosity index improver or in lieu of a viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt % to about 20 wt %, about 0.1 wt % to about 15 wt %, about 0.1 wt % to about 12 wt %, or about 0.5 wt % to about 10 wt %, of the lubricating oil composition.

Other Optional Additives: Other additives may be selected to perform one or more functions required of a lubricating fluid. Further, one or more of the mentioned additives may be multi-functional and provide functions in addition to or other than the function prescribed herein.

A lubricating oil composition according to the present disclosure may optionally comprise other performance additives. The other performance additives may be in addition to specified additives of the present disclosure and/or may comprise one or more of metal deactivators, viscosity index improvers, detergents, ashless TBN boosters, friction modifiers, antiwear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptothiadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers including trialkyl phosphates, polyethylene glycols, polyethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include polymethylmethacrylates or mixtures thereof. Pour point depressants may be present in an amount sufficient to provide from about 0 wt % to about 1 wt %, about 0.01 wt % to about 0.5 wt %, or about 0.02 wt % to about 0.04 wt % based upon the final weight of the lubricating oil composition.

Suitable rust inhibitors may be a single compound or a mixture of compounds having the property of inhibiting corrosion of ferrous metal surfaces. Non-limiting examples of rust inhibitors useful herein include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexadecenylsuccinic acid. Another useful type of acidic corrosion inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid.

The rust inhibitor, if present, can be used in an amount sufficient to provide about 0 wt % to about 5 wt %, about 0.01 wt % to about 3 wt %, about 0.1 wt % to about 2 wt %, based upon the final weight of the lubricating oil composition.

In general terms, a suitable lubricant including the detergent metals herein may include additive components in the ranges listed in the following table.

TABLE 2

| Suitable Lubricating Compositions      |                                 |                                 |
|----------------------------------------|---------------------------------|---------------------------------|
| Component                              | Wt. %<br>(Suitable Embodiments) | Wt. %<br>(Suitable Embodiments) |
| Detergent Systems                      | 0.02-5.0                        | 0.2-2.0                         |
| Dispersant(s)                          | 0-8.0                           | 1-6.0                           |
| Antioxidant(s)                         | 0.1-5.0                         | 0.01-3.0                        |
| Other Detergent(s)                     | 0.0-15.0                        | 0.2-8.0                         |
| Ashless TBN booster(s)                 | 0.0-1.0                         | 0.01-0.5                        |
| Corrosion inhibitor(s)                 | 0.0-5.0                         | 0.0-2.0                         |
| Metal dihydrocarbyldithiophosphate(s)  | 0.0-6.0                         | 0.1-4.0                         |
| Ash-free phosphorus compound(s)        | 0.0-6.0                         | 0.0-4.0                         |
| Antifoaming agent(s)                   | 0.0-5.0                         | 0.001-0.15                      |
| Antiwear agent(s)                      | 0.0-1.0                         | 0.0-0.8                         |
| Pour point depressant(s)               | 0.0-5.0                         | 0.01-1.5                        |
| Viscosity index improver(s)            | 0.0-25.0                        | 0.1-15.0                        |
| Dispersant viscosity index improver(s) | 0.0-10.0                        | 0.0-5.0                         |
| Friction modifier(s)                   | 0.00-5.0                        | 0.01-2.0                        |
| Base oil                               | Balance                         | Balance                         |
| Total                                  | 100                             | 100                             |

The percentages of each component above represent the weight percent of each component, based upon the weight of the final lubricating oil composition. The remainder of the lubricating oil composition consists of one or more base oils. Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). Fully formulated lubricants conventionally contain an additive package, referred to herein as a dispersant/inhibitor package or DI package, that will supply the characteristics that are required in the formulation.

#### DEFINITIONS

For purposes of this disclosure, the chemical elements are identified in accordance with the Periodic Table of the Elements, CAS version, Handbook of Chemistry and Physics, 75th Ed. Additionally, general principles of organic chemistry are described in "Organic Chemistry", Thomas Sorrell, University Science Books, Sausalito: 1999, and "March's Advanced Organic Chemistry", 5th Ed., Ed.: Smith, M. B. and March, J., John Wiley & Sons, New York: 2001, the entire contents of which are hereby incorporated by reference.

As described herein, compounds may optionally be substituted with one or more substituents, such as are illustrated generally above, or as exemplified by particular classes, subclasses, and species of the disclosure.

Unless otherwise apparent from the context, the term "major amount" is understood to mean an amount greater than or equal to 50 weight percent, for example, from about 80 to about 98 weight percent relative to the total weight of the composition. Moreover, as used herein, the term "minor amount" is understood to mean an amount less than 50 weight percent relative to the total weight of the composition.

As used herein, the term "hydrocarbyl group" or "hydrocarbyl" is used in its ordinary sense, which is well-known to those skilled in the art. Specifically, it refers to a group having a carbon atom directly attached to the remainder of a molecule and having a predominantly hydrocarbon character. Examples of hydrocarbyl groups include: (1) hydrocarbon substituents, that is, aliphatic (e.g., alkyl or alkenyl),

25 alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical); (2) substituted hydrocarbon substituents, that is, substituents containing non-hydrocarbon groups which, in the context of 30 the description herein, do not alter the predominantly hydrocarbon substituent (e.g., halo (especially chloro and fluoro), hydroxy, alkoxy, mercapto, alkylmercapto, nitro, nitroso, amino, alkylamino, and sulfoxy); (3) hetero-substituents, that is, substituents which, while having a predominantly 35 hydrocarbon character, in the context of this description, contain other than carbon in a ring or chain otherwise composed of carbon atoms. Hetero-atoms include sulfur, oxygen, nitrogen, and encompass substituents such as pyridyl, furyl, thieryl, and imidazolyl. In general, no more 40 than two, or as a further example, no more than one, non-hydrocarbon substituent will be present for every ten carbon atoms in the hydrocarbyl group; in some embodiments, there will be no non-hydrocarbon substituent in the hydrocarbyl group.

45 As used herein the term "aliphatic" encompasses the terms alkyl, alkenyl, alkynyl, each of which being optionally substituted as set forth below.

As used herein, an "alkyl" group refers to a saturated 50 aliphatic hydrocarbon group containing 1-12 (e.g., 1-8, 1-6, or 1-4) carbon atoms. An alkyl group can be straight or branched. Examples of alkyl groups include, but are not limited to, methyl, ethyl, propyl, isopropyl, butyl, isobutyl, sec-butyl, tert-butyl, n-pentyl, n-heptyl, or 2-ethylhexyl. An alkyl group can be substituted (i.e., optionally substituted) 55 with one or more substituents such as halo, phospho, cycloaliphatic [e.g., cycloalkyl or cycloalkenyl], heterocycloaliphatic [e.g., heterocycloalkyl or heterocycloalkenyl], aryl, heteroaryl, alkoxy, aryl, heteroaroyl, acyl [e.g., (aliphatic) carbonyl, (cycloaliphatic)carbonyl, or (heterocycloaliphatic) carbonyl], nitro, cyano, amido [e.g., (cycloalkylalkyl)carbonylamino, arylcarbonylamino, aralkylcarbonylamino, (heterocycloalkyl) carbonylamino, (heterocycloalkylalkyl) carbonylamino, heteroarylcarbonylamino, heteroaralkyl carbonylamino alkylaminocarbonyl, cycloalkylaminocarbonyl, heterocycloalkylaminocarbonyl, arylaminocarbonyl, or heteroarylaminocarbonyl], amino [e.g., aliphaticamino, cycloaliphatic amino, or heterocycloaliphaticamino], sulfonyl 60 65

[e.g., aliphatic-SO<sub>2</sub>—], sulfinyl, sulfanyl, sulfoxy, urea, thiourea, sulfamoyl, sulfamide, oxo, carboxy, carbamoyl, cycloaliphaticoxy, heterocyclo aliphaticoxy, aryloxy, heteroaryloxy, aralkyloxy, heteroarylalkoxy, alkoxy carbonyl, alkyl carbonyloxy, or hydroxy. Without limitation, some examples of substituted alkyls include carboxyalkyl (such as HOOC-alkyl, alkoxy carbonylalkyl, and alkyl carbonyloxy-alkyl), cyanoalkyl, hydroxylalkyl, alkoxyalkyl, acylalkyl, aralkyl, (alkoxyaryl)alkyl, (sulfonylamino) alkyl (such as (alkyl-SO<sub>2</sub>-amino)alkyl), aminoalkyl, amidoalkyl, (cycloaliphatic)alkyl, or haloalkyl.

As used herein, an “alkenyl” group refers to an aliphatic carbon group that contains 2-8 (e.g., 2-12, 2-6, or 2-4) carbon atoms and at least one double bond. Like an alkyl group, an alkenyl group can be straight or branched. Examples of an alkenyl group include, but are not limited to allyl, isoprenyl, 2-but enyl, and 2-hexenyl. An alkenyl group can be optionally substituted with one or more substituents such as halo, phospho, cycloaliphatic [e.g., cycloalkyl or cycloalkenyl], heterocycloaliphatic [e.g., heterocycloalkyl or hetero cycloalkenyl], aryl, heteroaryl, alkoxy, aroyl, heteroaroyl, acyl [e.g., (aliphatic) carbonyl, (cycloaliphatic) carbonyl, or (heterocycloaliphatic) carbonyl], nitro, cyano, amino [e.g., (cycloalkylalkyl)carbonylamino, arylcarbonylamino, aralkylcarbonylamino, (hetero cycloalkyl) carbonylamino, (heterocyclo alkylalkyl) carbonylamino, heteroarylcarbonylamino, heteroaralkylcarbonylamino alkylamino carbonyl, cycloalkylaminocarbonyl, hetero cyclo alkylaminocarbonyl, arylaminocarbonyl, or heteroarylamino carbonyl], amino [e.g., aliphaticamino, cycloaliphaticamino, heterocyclo aliphaticamino, or aliphatic sulfon酰amino], sulfonyl [e.g., alkyl-SO<sub>2</sub>—, cycloaliphatic-SO<sub>2</sub>—, or aryl-SO<sub>2</sub>—], sulfinyl, sulfanyl, sulfoxy, urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroaralkoxy, alkoxy carbonyl, alkyl carbonyloxy, or hydroxy. Without limitation, some examples of substituted alkenyls include cyanoalkenyl, alkoxyalkenyl, acylalkenyl, hydroxyl alkenyl, aralkenyl, (alkoxyaryl) alkenyl, (sulfonylamino)alkenyl (such as (alkyl-SO<sub>2</sub>-amino) alkenyl), aminoalkenyl, amidoalkenyl, (cycloaliphatic)alkenyl, or haloalkenyl.

As used herein, an “alkynyl” group refers to an aliphatic carbon group that contains 2-8 (e.g., 2-12, 2-6, or 2-4) carbon atoms and has at least one triple bond. An alkynyl group can be straight or branched. Examples of an alkynyl group include, but are not limited to, propargyl and butynyl. An alkynyl group can be optionally substituted with one or more substituents such as aroyl, heteroaroyl, alkoxy, cycloalkyloxy, heterocycloalkyloxy, aryloxy, heteroaryloxy, aralkyl oxy, nitro, carboxy, cyano, halo, hydroxy, sulfo, mercapto, sulfanyl [e.g., aliphatic sulfanyl or cycloaliphatic sulfanyl], sulfinyl [e.g., aliphatic sulfinyl or cycloaliphatic sulfinyl], sulfonyl [e.g., aliphatic-SO<sub>2</sub>—, aliphaticamino-SO<sub>2</sub>—, or cycloaliphatic-SO<sub>2</sub>—], amido [e.g., aminocarbonyl, alkylaminocarbonyl, alkylcarbonylamino, cyclo alkylaminocarbonyl, heterocycloalkylaminocarbonyl, cycloalkylcarbonylamino, arylamino carbonyl, arylcarbonylamino, aralkylcarbonylamino, (heterocycloalkyl) carbonylamino, (cycloalkylalkyl) carbonylamino, heteroaralkylcarbonylamino, heteroaryl carbonylamino or heteroaryl amino carbonyl], urea, thiourea, sulfamoyl, sulfamide, alkoxy carbonyl, alkyl carbonyloxy, cyclo aliphatic, heterocycloaliphatic, aryl, heteroaryl, acyl [e.g., (cycloaliphatic) carbonyl or (hetero cyclo aliphatic) carbonyl], amino [e.g.,

aliphaticamino], sulfoxy, oxo, carboxy, carbamoyl, (cycloaliphatic)oxy, (heterocyclo aliphatic) oxy, or (heteroaryl) alkoxy.

As used herein, an “amino” group refers to —NR<sup>X</sup>R<sup>Y</sup> where in each of R<sup>X</sup> and R<sup>Y</sup> is independently hydrogen, alkyl, cycloalkyl, (cycloalkyl)alkyl, aryl, aralkyl, heterocycloalkyl, (heterocycloalkyl)alkyl, heteroaryl, carboxy, sulfanyl, sulfinyl, sulfonyl, (alkyl)carbonyl, (cycloalkyl)carbonyl, ((cycloalkyl)alkyl)carbonyl, arylcarbonyl, (aralkyl)carbonyl, (heterocyclo alkyl) carbonyl, ((heterocycloalkyl)alkyl)carbonyl, (heteroaryl)carbonyl, or (heteroaralkyl) carbonyl, each of which being defined herein and being optionally substituted. Examples of amino groups include alkylamino, dialkylamino, or arylamino. When the term “amino” is not the terminal group (e.g., alkylcarbonylamino), it is represented by —NR<sup>X</sup>—. R<sup>X</sup> has the same meaning as defined above.

As used herein, a “cycloalkyl” group refers to a saturated carbocyclic mono- or bicyclic (fused or bridged) ring of 3-10 (e.g., 5-10) carbon atoms. Examples of cycloalkyl groups include cyclopropyl, cyclobutyl, cyclopentyl, cyclohexyl, cycloheptyl, adamantyl, norbornyl, cubyl, octahydroindenyl, decahydro-naphthyl, bicyclo[3.2.1]octyl, bicyclo[2.2.2]octyl, bicyclo[3.3.1]nonyl, bicyclo[3.3.2.]decyl, bicyclo[2.2.2]octyl, adamantyl, or ((aminocarbonyl)cycloalkyl)cycloalkyl.

As used herein, a “heterocycloalkyl” group refers to a 3-10 membered mono- or bicyclic (fused or bridged) (e.g., 5- to 10-membered mono- or bicyclic) saturated ring structure, in which one or more of the ring atoms is a heteroatom (e.g., N, O, S, or combinations thereof). Examples of a heterocycloalkyl group include piperidyl, piperazyl, tetrahydropyranyl, tetrahydrofuryl, 1,4-dioxolanyl, 1,4-dithianyl, 1,3-dioxolanyl, oxazolidyl, isoxazolidyl, morpholinyl, thiomorpholyl, octahydrobenzofuryl, octahydrochromenyl, octahydrothio chromenyl, octahydroindolyl, octahydropyridinyl, decahydroquinolinyl, octahydrobenzo[b] thienophenyl, 2-oxa-bicyclo[2.2.2]octyl, 1-aza-bicyclo[2.2.2]octyl, 3-aza-bicyclo[3.2.1]octyl, and 2,6-dioxa-tricyclo[3.3.1.0]nonyl. A monocyclic heterocycloalkyl group can be fused with a phenyl moiety to form structures, such as tetrahydroisoquinoline, which would be categorized as heteroaryls.

A “heteroaryl” group, as used herein, refers to a monocyclic, bicyclic, or tricyclic ring system having 4 to 15 ring atoms wherein one or more of the ring atoms is a heteroatom (e.g., N, O, S, or combinations thereof) and in which the monocyclic ring system is aromatic or at least one of the rings in the bicyclic or tricyclic ring systems is aromatic. A heteroaryl group includes a benzofused ring system having 2 to 3 rings. For example, a benzofused group includes benzo fused with one or two 4 to 8 membered heterocycloaliphatic moieties (e.g., indolizyl, indolyl, isoindolyl, 3H-indolyl, indolinyl, benzo[b]furyl, benzo[b]thiophenyl, quinolinyl, or isoquinolinyl). Some examples of heteroaryl are pyridyl, 1H-indazolyl, furyl, pyrrolyl, thienyl, thiazolyl, oxazolyl, imidazolyl, tetrazolyl, benzofuryl, isoquinolinyl, benzthiazolyl, xanthene, thioxanthene, phenothiazine, dihydroindole, benzo[1,3]dioxole, benzo[b]furyl, benzo[b] thienophenyl, indazolyl, benzimidazolyl, benzthiazolyl, puryl, cinnolyl, quinolyl, quinazolyl, cinnolyl, phthalazyl, quinazolyl, quinoxalyl, isoquinolyl, 4H-quinolizyl, benzo-1,2,5-thiadiazolyl, or 1,8-naphthyridyl.

Without limitation, monocyclic heteroaryls include furyl, thiophenyl, 2H-pyrrolyl, pyrrolyl, oxazolyl, thiazolyl, imidazolyl, pyrazolyl, isoxazolyl, isothiazolyl, 1,3,4-thiadiazolyl, 2H-pyranyl, 4H-quinolizyl, pyridyl, pyridazyl, pyrimidyl,

pyrazolyl, pyrazyl, or 1,3,5-triazyl. Monocyclic heteroaryls are numbered according to standard chemical nomenclature.

Without limitation, bicyclic heteroaryls include indolizyl, indolyl, isoindolyl, 3H-indolyl, indolinyl, benzo[b]furyl, benzo[b]thiophenyl, quinolinyl, isoquinolinyl, indolizinyl, isoindolyl, indolyl, benzo[b]furyl, bexo[b]thiophenyl, indazolyl, benzimidazyl, benzthiazolyl, purinyl, 4H-quinolizyl, quinolyl, isoquinolyl, cinnolyl, phthalazyl, quinazolyl, quinoxalyl, 1,8-naphthyridyl, or pteridyl. Bicyclic heteroaryls are numbered according to standard chemical nomenclature.

As used herein, the term "treat rate" refers to the weight percent of a component in the lubricating and cooling fluids.

The weight average molecular weight (Mw) and the number average molecular weight (Mn) may be determined with a gel permeation chromatography (GPC) instrument obtained from Waters or the like instrument and the data processed with Waters Empower Software or the like software. The GPC instrument may be equipped with a Waters Separations Module and Waters Refractive Index detector (or the like optional equipment). The GPC operating conditions may include a guard column, 4 Agilent PLgel columns (length of 300×7.5 mm; particle size of 5 $\mu$ , and pore size ranging from 100-10000 Å) with the column temperature at about 40° C. Un-stabilized HPLC grade tetrahydrofuran (THF) may be used as solvent, at a flow rate of 1.0 mL/min. The GPC instrument may be calibrated with commercially available poly(methyl methacrylate) (PMMA) standards having a narrow molecular weight distribution ranging from 960-1,568,000 g/mol. The calibration curve can be extrapolated for samples having a mass less than 500 g/mol. Samples and PMMA standards can be in dissolved in THF and prepared at concentration of 0.1 to 0.5 wt. % and used without filtration. GPC measurements are also described in U.S. Pat. No. 5,266,223, which is incorporated herein by reference. The GPC method additionally provides

## EXAMPLES

A better understanding of the present disclosure and its many advantages may be clarified with the following examples. The following examples are illustrative and not limiting thereof in either scope or spirit. Those skilled in the art will readily understand that variations of the components, methods, steps, and devices described in these examples can be used. Unless noted otherwise or apparent from the context of discussion in the Examples below and throughout this disclosure, all percentages, ratios, and parts noted in this disclosure are by weight.

Various lubricating compositions were evaluated for piston cleanliness pursuant to CEC L-117-20 (TDi3) and fuel economy performance pursuant to JASO M 366. Each lubricating composition evaluated for this Example included a similar additive package of dispersants, antiwear additives, aminic antioxidants, phenolic antioxidants, molybdenum antioxidants, friction modifiers, antifoam agents, pour point depressants and process oil contributing about 1300 ppm of magnesium, about 40 ppm of molybdenum, about 780 ppm of phosphorus, about 1700 ppm of sulfur, and about 860 ppm of zinc to the lubricant. The additive package also had a detergent TBN (ASTM 4739) of about 5.7 mg KOH/gram and a calculated SASH (ASTM D874) of about 0.75 wt %.

The additive package was blended into lubricating compositions set forth in Table 3 below including a molybdenum dialkyl dithiocarbamate compound and a polymethacrylate viscosity index improver. Each lubricant also included a base oil blend selected from Group III base oils of about 4 to about 8 cSt and Group IV. Table 3 also provides further details on the lubricants including the VW TDi3 piston cleanliness results and the JASO fuel economy improvements. Fuel economy was conducted on a Toyota 2ZR-FXE engine (e.g., Toyota Prius, 1.8 L, inline 5, port fuel injection)

TABLE 3

| Fluid Relationships and Performance     |             |             |             |
|-----------------------------------------|-------------|-------------|-------------|
|                                         | Inventive 1 | Inventive 2 | Inventive 3 |
| Oil-soluble Molybdenum compound, Mo ppm | 600         | 600         | 600         |
| PMA Copolymer, %                        | 4.70        | 4.00        | —           |
| 4 to 8 cSt Group III base oil(s)        | —           | Balance     | Balance     |
| 4 cSt Group IV Base oil(s)              | Balance     | —           | —           |
| Mg, ppm                                 | 1218        | 1221        | 1346        |
| Mo, ppm                                 | 607         | 607         | 613         |
| P, ppm                                  | 765         | 764         | 804         |
| S, ppm                                  | 2418        | 2417        | 2504        |
| Zn, ppm                                 | 860         | 857         | 867         |
| N, ppm                                  | 1300        | 1300        | 1210        |
| SASH, % (D874)                          | 0.81%       | 0.84%       | 0.73%       |
| TBN, mg KOH/g (D2896)                   | 8.6         | 8.6         | 8.7         |
| TBN, mg KOH/g (D4739)                   | 6.5         | 6.6         | 6.4         |
| KV100, cSt (D445)                       | 6.33        | 6.35        | 6.63        |
| KV40, cSt (D445)                        | 27.35       | 27.80       | 34.89       |
| BOV 100, cSt (D445)                     | 4.00        | 4.16        | 5.14        |
| VI                                      | 195         | 191         | 149         |
| CCS -35 (D5292)                         | 2414        | 3284        | 5441        |
| HTHS 150                                | 2.26        | 2.26        | 2.28        |
| HTHS 100                                | 4.47        | 4.53        | 5.15        |
| NOACK 250, % (CEC L-40-93)              | 11.2        | 11.2        | 7.9         |
| VW TDi3 (CECL-117-20)                   | —           | 53 merits   | 59 merits   |
| JASO M 366 FE                           | 0.87%       | 0.87%       | 0.53%       |

— HTHS is measured via one of D4683, D4741, or D5471

molecular weight distribution information; see, for example, W. W. Yau, J. J. Kirkland and D. D. Bly, "Modern Size Exclusion Liquid Chromatography", John Wiley and Sons, New York, 1979, also incorporated herein by reference.

It is noted that, as used in this specification and the appended claims, the singular forms "a," "an," and "the," include plural referents unless expressly and unequivocally limited to one referent. Thus, for example, reference to "an

“antioxidant” includes two or more different antioxidants. As used herein, the term “include” and its grammatical variants are intended to be non-limiting, such that recitation of items in a list is not to the exclusion of other like items that can be substituted or added to the listed items

For the purposes of this specification and appended claims, unless otherwise indicated, all numbers expressing quantities, percentages or proportions, and other numerical values used in the specification and claims, are to be understood as being modified in all instances by the term “about.” Accordingly, unless indicated to the contrary, the numerical parameters set forth in the following specification and attached claims are approximations that can vary depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques.

It is to be understood that each component, compound, substituent or parameter disclosed herein is to be interpreted as being disclosed for use alone or in combination with one or more of each and every other component, compound, substituent or parameter disclosed herein.

It is further understood that each range disclosed herein is to be interpreted as a disclosure of each specific value within the disclosed range that has the same number of significant digits. Thus, for example, a range from 1 to 4 is to be interpreted as an express disclosure of the values 1, 2, 3 and 4 as well as any range of such values.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range. That is, it is also further understood that any range between the endpoint values within the broad range is also discussed herein. Thus, a range from 1 to 4 also means a range from 1 to 3, 1 to 2, 2 to 4, 2 to 3, and so forth.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications variations, improvements, and substantial equivalents.

What is claimed is:

1. An engine lubricating oil composition for lubricating a diesel internal combustion engine, the engine lubricating oil composition comprising:

one or more base oils of lubricating viscosity, wherein the one or more base oils have a combined base oil viscosity at 100° C. of less than or equal to about 5.4 cSt;

5 a detergent system providing a minimum total base number (TBN), measured pursuant to ASTM D4739, to the engine lubricating oil composition of at least about 4 to about 7 mg KOH/g, and wherein the detergent system includes only a magnesium-containing detergent additive;

wherein the engine lubricating oil composition has (i) a NOACK volatility of about 13% or less measured pursuant to CEC L-40-90 and/or ASTM D5800; (ii) a total base number (TBN) of the engine lubricating oil composition of about 7 to about 9 mg KOH/g measured pursuant to ASTM D2896; (iii) a calculated sulfated ash content (SASH) of about 0.8 weight percent or less measured pursuant to ASTM D874; and (iv) a CCS viscosity at -35° C. of about 6200 mPas or less measured pursuant to ASTM D5292.

2. The engine lubricating oil composition of claim 1, wherein the engine lubricating oil composition meets or exceeds lubricant performance set forth in the CEC L-117-20 (VW TDi3) piston cleanliness test with a piston cleanliness rating of at least about 53 merits.

3. The engine lubricating oil composition of claim 2, wherein the engine lubricating oil composition has a positive fuel economy increase as measured pursuant to JASO M 366 of at least about 0.5%.

30 4. The engine lubricating oil composition of claim 1, wherein the detergent system is substantially free of phenate detergent additives and wherein the detergent system consists essentially of sulfonate detergent additives.

5. The engine lubricating oil composition of claim 1, 35 wherein the detergent system provides about 800 to about 1800 ppm of magnesium to the engine lubricating oil composition.

6. The engine lubricating oil composition of claim 1, 40 wherein the detergent system includes one or more over-based detergent additives having a total base number (TBN) as measured pursuant to ASTM D2896 of at least about 250 mg KOH/g.

7. The engine lubricating oil composition of claim 1, 45 wherein the engine lubricating oil composition has a TBN of about 8 or less measured pursuant to ASTM D2896.

8. The engine lubricating oil composition of claim 1, further comprising an oil-soluble molybdenum containing additive providing no more than about 800 ppm of molybdenum to the engine lubricating oil composition.

50 9. The engine lubricating oil composition of claim 1, further comprising about 2 to about 10 weight percent of one or more polymeric viscosity index improver additives.

10. The engine lubricating oil composition of claim 9, 55 wherein the engine lubricating oil composition has a viscosity index of 130 to 300.

11. The engine lubricating oil composition of claim 10, wherein the one or more polymeric viscosity index improver additive is one of (i) an olefin copolymer, (ii) a dispersant or a non-dispersant poly (meth)acrylate copolymer viscosity modifier having a weight average molecular weight of about 500,000 or less, or (iii) combinations thereof.

12. The engine lubricating oil composition of claim 11, 60 wherein the one or more polymeric viscosity index improver additive is the dispersant or the non-dispersant poly (meth)acrylate copolymer and has a weight average molecular weight of about 200,000 to about 500,000 with a polydispersity index of about 1.5 to about 2.5 and includes first

39

(meth)acrylate monomer units with a hydrocarbyl group in a monomer ester moiety of up to about 700 and second (meth)acrylate monomer units with a hydrocarbyl group in a monomer ester moiety of up to about 10000.

13. The engine lubricating oil composition of claim 1, wherein the engine lubricating oil composition has a viscosity grade of 0W-X, wherein X is 8, 12, 16, 20, or 30.

14. The engine lubricating oil composition of claim 13, wherein the base oil viscosity is about 5.2 cSt or less.

15. The engine lubricating oil composition of claim 1, wherein the engine lubricating oil composition is substantially free of boron, substantially free of calcium, or combinations thereof.

16. The engine lubricating oil composition of claim 1, further including one or more metal dihydrocarbyl dithiophosphate compounds, and wherein the one or more metal dihydrocarbyl dithiophosphate compounds provide up to about 1000 ppm phosphorus to the lubricating oil composition.

17. The engine lubricating oil composition of claim 1, further comprising one or more sulfur-containing additives, and wherein the one or more sulfur-containing additives provide up to about 2500 ppm sulfur to the lubricating oil composition.

18. A method of improving the fuel economy and the piston cleanliness of a passenger car diesel engine using a lubricating oil composition, the method comprising:

40

lubricating an engine crankcase of a passenger car diesel engine with a lubricating oil composition; wherein the lubricating oil composition is set forth in claim 1; and

wherein the lubricating oil composition meets or exceeds lubricant performance set forth in the CEC L-117-20 (VW TDi3) piston cleanliness test with a piston cleanliness rating of at least about 53 merits and the lubricating oil composition has a positive fuel economy increase as measured pursuant to JASO M 366 with a fuel economy improvement of at least about 0.5%.

19. A method of lubricating a crankcase of a passenger car diesel engine using a lubricating oil composition, the method comprising:

lubricating an engine crankcase of a passenger car diesel engine with a lubricating oil composition; wherein the lubricating oil composition is set forth in claim 1; and

wherein the passenger car engine lubricated with the lubricating oil composition meets or exceeds lubricant performance set forth in the CEC L-117-20 (VW TDi3) piston cleanliness test with a piston cleanliness rating of at least about 53 merits and has a positive fuel economy increase as measured pursuant to JASO M 366 with a fuel economy improvement of at least about 0.5%.

\* \* \* \* \*